



US012195695B2

(12) **United States Patent**  
**Yang et al.**

(10) **Patent No.:** **US 12,195,695 B2**  
(45) **Date of Patent:** **Jan. 14, 2025**

(54) **LUBRICATING OIL COMPOSITIONS FOR IMPROVING LOW-SPEED PRE-IGNITION**

(71) Applicant: **Afton Chemical Corporation**, Richmond, VA (US)

(72) Inventors: **Kongsheng Yang**, Glen Allen, VA (US); **Brent Calcut**, Detroit, MI (US); **Amy M. James**, Richmond, VA (US); **Kristi Engelman**, Richmond, VA (US)

(73) Assignee: **Afton Chemical Corporation**, Richmond, VA (US)

(\*) Notice: Subject to any disclaimer, the term of this patent is extended or adjusted under 35 U.S.C. 154(b) by 0 days.

(21) Appl. No.: **18/315,013**

(22) Filed: **May 10, 2023**

(65) **Prior Publication Data**

US 2024/0376395 A1 Nov. 14, 2024

(51) **Int. Cl.**

**C10M 169/04** (2006.01)  
**C10M 135/10** (2006.01)  
**C10M 137/10** (2006.01)  
**C10M 141/10** (2006.01)  
**C10M 155/02** (2006.01)  
**C10M 161/00** (2006.01)  
**C10N 30/00** (2006.01)  
**C10N 30/04** (2006.01)  
**C10N 40/25** (2006.01)

(52) **U.S. Cl.**

CPC ..... **C10M 169/044** (2013.01); **C10M 135/10** (2013.01); **C10M 137/10** (2013.01); **C10M 141/10** (2013.01); **C10M 155/02** (2013.01); **C10M 161/00** (2013.01); **C10M 2203/003** (2013.01); **C10M 2219/044** (2013.01); **C10M 2223/045** (2013.01); **C10M 2229/041** (2013.01); **C10N 2030/041** (2020.05); **C10N 2030/52** (2020.05); **C10N 2040/255** (2020.05)

(58) **Field of Classification Search**

CPC ..... C10M 169/044; C10M 135/10; C10M 137/10; C10M 141/10; C10M 155/02; C10M 161/00; C10M 2203/003; C10M 2219/044; C10M 2223/045; C10M 2229/041

See application file for complete search history.

(56) **References Cited**

U.S. PATENT DOCUMENTS

3,502,677 A 3/1970 Lesner  
3,697,429 A 10/1972 Engel et al.  
3,763,244 A 10/1973 Shubkin  
3,816,346 A 6/1974 Coppock et al.

3,991,056 A 11/1976 Okamoto et al.  
4,036,771 A 7/1977 Denis et al.  
4,118,329 A 10/1978 Hotten  
4,234,435 A 11/1980 Meinhardt et al.  
4,282,392 A 8/1981 Cupples et al.  
4,285,822 A 8/1981 deVries et al.  
4,537,696 A 8/1985 Beimesch  
4,587,368 A 5/1986 Pratt  
4,747,971 A 5/1988 Erdman  
4,857,214 A 8/1989 Papay et al.  
4,925,983 A 5/1990 Steckel  
4,941,984 A 7/1990 Chamberlin, III et al.  
4,956,122 A 9/1990 Watts et al.  
4,992,183 A 2/1991 Beimesch et al.  
5,089,156 A 2/1992 Chrisope et al.  
5,114,602 A 5/1992 Petrille et al.  
5,614,480 A 3/1997 Salomon et al.  
6,124,247 A 9/2000 Cazin et al.  
6,303,546 B1 10/2001 Hata et al.  
8,260,530 B2 9/2012 Rollinger et al.  
8,327,687 B2 12/2012 Amann et al.  
8,543,315 B2 9/2013 Glugla et al.  
11,034,912 B2 6/2021 Ritchie et al.  
2002/0165102 A1 11/2002 Hata et al.  
2004/0242434 A1 12/2004 Yagishita et al.  
2005/0101496 A1 5/2005 Loper et al.  
2006/0058200 A1 3/2006 Shaw et al.

(Continued)

FOREIGN PATENT DOCUMENTS

EP 0088453 A1 9/1983  
EP 1788068 A1 5/2007  
(Continued)

OTHER PUBLICATIONS

Takeuchi et al., Investigation of Engine Oil Effect on Abnormal Combustion in Turbocharged Direct Injection-Spark Ignition Engines, SAE Int., Nov. 2012, vol. 5, Issue 3.(Abstract).

(Continued)

Primary Examiner — Vishal V Vasisth

(74) Attorney, Agent, or Firm — Honigman LLP

(57) **ABSTRACT**

The present disclosure relates to lubricating compositions and methods of lubricating a spark-ignition engine effective to improve low-speed pre-ignition (LSPI) through selection of lubricant elemental relationships rather than through the addition of supplemental fluid additives with the added benefit that the relationships herein, in some circumstances, improve the low-speed pre-ignition independent of the underlying base oil quality. The lubricating compositions herein include one or more base oils of lubricating viscosity, one or more phosphorus-containing additives providing low levels of phosphorus, a detergent system providing calcium and/or magnesium with certain relationships of the calcium sulfated ash content to the low phosphorus content.

| (56)                     | References Cited |                 |             |                |         |  |
|--------------------------|------------------|-----------------|-------------|----------------|---------|--|
| U.S. PATENT DOCUMENTS    |                  |                 |             |                |         |  |
| 2006/0217271 A1          | 9/2006           | Brown et al.    | GB          | 961009 A       | 6/1964  |  |
| 2007/0184992 A1          | 8/2007           | Takeuchi et al. | JP          | 2014152301 A   | 8/2014  |  |
| 2008/0128184 A1          | 6/2008           | Loper et al.    | JP          | 2016534216 A   | 11/2016 |  |
| 2009/0156446 A1          | 6/2009           | McAtee et al.   | JP          | 2017514984 A   | 6/2017  |  |
| 2011/0111997 A1          | 5/2011           | Cook et al.     | WO          | 2009104682 A1  | 8/2009  |  |
| 2011/0213538 A1          | 9/2011           | Amann et al.    | WO          | 2015023559 A1  | 2/2015  |  |
| 2011/0265761 A1          | 11/2011          | Amann et al.    | WO          | 2015042337 A1  | 3/2015  |  |
| 2012/0029789 A1          | 2/2012           | Mehta et al.    | WO          | 2015042340 A1  | 3/2015  |  |
| 2012/0186225 A1          | 7/2012           | Amann et al.    | WO          | 2015042341 A1  | 3/2015  |  |
| 2013/0035841 A1          | 2/2013           | Glugla et al.   | WO          | 2015076417 A1  | 5/2015  |  |
| 2015/0322367 A1          | 11/2015          | Patel et al.    | WO          | 20150114920 A1 | 8/2015  |  |
| 2015/0322369 A1          | 11/2015          | Patel et al.    | WO          | 2017011691 A1  | 1/2017  |  |
| 2016/0230116 A1          | 8/2016           | Mosier et al.   | WO          | 2020085228 A1  | 4/2020  |  |
| 2017/0015926 A1          | 1/2017           | Fletcher et al. |             |                |         |  |
| 2017/0015930 A1          | 1/2017           | Fletcher        |             |                |         |  |
| 2017/0022441 A1          | 1/2017           | Onodera         |             |                |         |  |
| 2021/0371767 A1*         | 12/2021          | Shimizu .....   | C10M 141/10 |                |         |  |
| 2021/0403824 A1*         | 12/2021          | Kikabhai .....  | C10M 129/74 |                |         |  |
| FOREIGN PATENT DOCUMENTS |                  |                 |             |                |         |  |
| EP                       | 2298855 A1 *     | 3/2011 .....    | C10M 143/06 |                |         |  |
| EP                       | 2639433 A1       | 9/2013          |             |                |         |  |

## OTHER PUBLICATIONS

Haenel et al., Systematic Approach to Analyze and Characterize Pre-ignition Events in Turbocharged Direct-injected Gasoline Engines, SAE Int., Apr. 2011.(Abstract).

\* cited by examiner

## 1

## LUBRICATING OIL COMPOSITIONS FOR IMPROVING LOW-SPEED PRE-IGNITION

## TECHNICAL FIELD

The present disclosure relates to lubricating compositions and, in particular, lubricating compositions configured to improve low-speed pre-ignition with lower levels of phosphorus.

## BACKGROUND

Automotive manufacturers continue to the push for improved efficiency, fluid longevity, and fuel economy, and as such, demands on engines, lubricants, and their components continue to increase. Today's engines are often smaller, lighter and more efficient with technologies designed to improve fuel economy, performance, and power. These requirements also mean engine oil performance must evolve to meet the higher demands of such modern engines and their corresponding performance criteria tied to their unique use and applications. With such exacting demands for engine oils, lubricant manufacturers often tailor lubricants and their additives to meet certain performance requirements for industry and/or manufacturer applications. Typically, industry standards and/or automotive manufacturers require certain performance standards such that a lubricant designed for one use or application may not satisfy all the performance specifications for a different use or application.

For example, the American Petroleum Institute (API) sets standards for passenger car motor oils designed to meet the needs and performance characteristics of various passenger car automobile manufacturers. Recent updates to API standards include performance testing relating to an undesired phenomenon typically characterized as low-speed pre-ignition (or LSPI), which is believed to be a form of combustion that results with ignition of the air-fuel mixture in the combustion chamber prior to the desired ignition. LSPI is evaluated pursuant to the Sequence IX low speed pre-ignition test as set forth in ASTM D8291-21a. Often, turbocharged or supercharged engines, may be prone to LSPI, which is a pre-ignition event that may include high pressure spikes, early combustion, and/or knock. A premature ignition in the combustion chamber, generated prior to the spark plug firing, may cause an abnormal combustion and high cylinder pressure. The LSPI event may result in a knocking sound or other abnormal characteristics from the uncontrolled pressure rise in the cylinder. LSPI events are undesired and recent API specifications set LSPI performance 47986063.1 standards for passenger car motor oils. Prior solutions to undesired LSPI events are less than satisfactory because fluid manufacturers tended to address LSPI problems with the addition of supplemental fluid componentry, which often places other constraints on the additive package in the fluid not to mention that supplemental additives can, in some instances, provide other unintended effects.

## SUMMARY

In one approach or embodiment, the present disclosure relates to a lubricating composition for a spark-ignition engine to provide good LSPI performance with low levels of phosphorus. In one aspect of this embodiment, the lubricating composition included one or more base oils of lubricating viscosity: one or more phosphorus-containing additives providing no more than about 500 ppm of phosphorus to the

## 2

lubricating composition: a detergent system providing one or more calcium-containing detergents and optionally one or more magnesium-containing detergents, and wherein the detergent system is substantially free of sodium-containing detergents: wherein the lubricating composition includes a calcium content such that the lubricating composition has no more than about 0.2 weight percent of calculated calcium sulfated ash content; and a weight ratio of phosphorus content to calcium sulfated ash content of at least about 0.1.

10 In other approaches or embodiments, the lubricating composition of the previous paragraph may include one or more optional features or embodiments in any combination. These optional features or embodiments may include one or more of the following: wherein the weight ratio of the phosphorus content to the calcium sulfated ash content is about 0.1 to about 0.3; and/or wherein the lubricating composition has a total calculated sulfated ash content (SASH) of about 1 weight percent or less; and/or wherein the lubricating composition has a total calculated sulfated ash content (SASH) of about 0.8 weight percent or less; and/or wherein the lubricating composition has a total calculated sulfated ash content (SASH) of about 0.7 weight percent or less; and/or wherein about 30 weight percent or less of the total calculated SASH content is provided by the calcium sulfated ash content; and/or further comprising one or more silicon-containing compounds providing about 3 to about 20 ppm silicon to the lubricating composition; and/or wherein the one or more silicon-containing compounds provide about 5 to about 15 ppm silicon; and/or wherein a weight ratio of calcium sulfated ash content to silicon content is about 250 or less; and/or wherein the silicon-containing compound is selected from organosilane compounds, fluorosilicone compounds, polydimethylsiloxane compounds, phenyl-methyl polysiloxane compounds, linear siloxane compounds, cyclic siloxane compounds, branched siloxane compounds, silicone polymers and copolymers, organo-silicone copolymers, silicone oil, or combinations thereof; and/or wherein the detergent system includes the calcium-containing detergent and the magnesium-containing detergent; and/or wherein the detergent system includes calcium sulfonate and optionally magnesium sulfonate; and/or wherein the calcium sulfonate and the optional magnesium sulfonate are each overbased and each having a total base number (TBN) of at least about 250 mg KOH/g as determined by ASTM D2896; and/or wherein the detergent system is free of phenate-based detergents; and/or wherein the one or more base oils of lubricating viscosity are selected from API Group I base oils, API Group II base oils, API Group III base oils, or combinations thereof; and/or wherein the one or more base oils of lubricating viscosity are selected from API Group I base oils, API Group II base oils, or combinations thereof; and/or wherein the lubricating composition exhibits no more than 5 average events pursuant to a Sequence IX low speed pre-ignition test of ASTM D8291 and/or exhibits no more than 8 maximum events pursuant to the Sequence IX low speed pre-ignition test of ASTM D8291; and/or wherein the one or more phosphorus-containing additives provide about 200 to about 400 ppm phosphorus.

60 In yet further approaches or embodiments, methods of lubricating a spark-ignition engine with a low phosphorus content lubricant is provided herein. In one aspect, the method includes lubricating the crankcase of a spark-ignition engine with a lubricating composition; wherein the lubricating composition includes (i) one or more base oils of lubricating viscosity: (ii) one or more phosphorus-containing additives providing no more than about 500 ppm of

phosphorus to the lubricating composition: (iii) a detergent system providing one or more calcium-containing detergents and optionally one or more magnesium-containing detergents, and wherein the detergent system is substantially free of sodium-containing detergents: (iv) wherein the lubricating composition includes a calcium content providing no more than about 0.2 weight percent of calculated calcium sulfated ash content; and (v) a weight ratio of phosphorus content to calcium sulfated ash content of at least about 0.1; and wherein the lubricating composition exhibits no more than 5 average events pursuant to a Sequence IX low speed pre-ignition test of ASTM D8291 and/or exhibits no more than 8 maximum events pursuant to the Sequence IX low speed pre-ignition test of ASTM D8291.

In further approaches or embodiments, the methods of the previous paragraph may include one or more optional steps, features, or embodiments in any combination. These optional steps, features, or embodiments may include more or more of the following: wherein the weight ratio of the phosphorus content to the calcium sulfated ash content is about 0.1 to about 0.3; and/or wherein the lubricating composition further includes one or more silicon-containing compounds providing about 3 to about 20 ppm silicon to the lubricating composition; and/or wherein a weight ratio of calcium sulfated ash content to silicon content is about 250 or less. The methods herein may also include any embodiment of the lubricating composition as described in this Summary.

In yet other approaches or embodiments, the present application further includes the use of a lubricating compositions having low levels of phosphorus to achieve passing LSPI pursuant to ASTM D8291. In aspects, the use includes lubricating the crankcase of a spark-ignition engine with a lubricating composition: wherein the lubricating composition includes (i) one or more base oils of lubricating viscosity: (ii) one or more phosphorus-containing additives providing no more than about 500 ppm of phosphorus to the lubricating composition: (iii) a detergent system providing one or more calcium-containing detergents and optionally one or more magnesium-containing detergents, and wherein the detergent system is substantially free of sodium-containing detergents: (iv) wherein the lubricating composition includes no more than about 0.2 weight percent of calculated calcium sulfated ash content; and (v) a weight ratio of phosphorus content to calcium sulfated ash content of at least about 0.1; and wherein the lubricating composition exhibits no more than 5 average events pursuant to a Sequence IX low speed pre-ignition test of ASTM D8291 and/or exhibits no more than 8 maximum events pursuant to the Sequence IX low speed pre-ignition test of ASTM D8291. The use herein may include any embodiment of the lubricating compositions has described in this Summary.

#### DETAILED DESCRIPTION

The present disclosure relates to lubricating compositions and methods of lubricating a spark-ignition engine effective to improve low-speed pre-ignition (LSPI) through selection of lubricant elemental relationships rather than through the addition of supplemental fluid additives with the added benefit that the relationships herein, in some circumstances, improve the low-speed pre-ignition independent of the underlying base oil quality. In approaches or embodiments, the lubricating compositions herein include one or more base oils of lubricating viscosity, one or more phosphorus-containing additives providing no more than about 500 ppm of phosphorus, a detergent system providing calcium and/or

magnesium that is substantially free of sodium-containing detergents, a calcium content providing no more than 0.2 weight percent of calcium sulfated ash content (Ca-SASH) as determined by ASTM D874 and/or preferably as calculated herein, and with a specific weight ratio of the phosphorus content to the calcium sulfated ash content in the lubricant of at least about 0.1 (and preferably about 0.1 to about 0.3). In yet other embodiments, the lubricant herein may also have unique relationships between the calcium sulfated ash and silicon in the lubricant where a weight ratio of the calcium sulfated ash content to the silicon content is about 250:1 or less (and in some approaches, about 100:1 to about 250:1).

Surprisingly, such discovered elemental relationships in the lubricants herein, and in particular, at least the phosphorus content relative to the calcium SASH content aids in achieving the low number of average and/or total LSPI events even with less total phosphorus than conventionally used in such lubricants and while maintaining a calcium content in the fluid. Previously, it has been known that calcium tended to be detrimental to LSPI (in view of the associated calcium sulfated ash content) and it was generally accepted that relatively high levels of phosphorus were beneficial for LSPI. The lubricants herein, on the other hand, go against this conventional practice by (1) lowering the amount of total phosphorus and (2) maintaining a calcium content in the lubricant that unexpectedly achieves desired LSPI performance when the elemental relationships associated with the phosphorus content, the calcium ash content and/or the silicon content are maintained within the ranges noted herein.

In some embodiments, the lubricating compositions herein with the above discovered elemental relationships exhibit no more than 5 average LSPI events pursuant to the Sequence IX low-speed pre-ignition test of ASTM D8291 (and in other approaches, no more than 4 average events, no more than 3 average event, no more than 2 average events, or no more than 1 average LSPI events). In other embodiments, the lubricating compositions herein exhibit no more than 8 total LSPI events pursuant to the Sequence IX low-speed pre-ignition test of ASTM D8291 (and in other approaches, no more than 7 total events, no more than 6 total events, no more than 5 total event, no more than 4 total events, no more than 3 total events, or no more than 2 total events).

#### Phosphorus-Containing Additives

The lubricating compositions herein include one or more phosphorus-containing additives in low amounts to provide no more than about 500 ppm of total phosphorus to the lubricants, and in other embodiments, no more than about 450 ppm of total phosphorus, no more than about 400 ppm of total phosphorus, no more than about 350 ppm of total phosphorus, no more than about 300 ppm of total phosphorus, or no more than about 250 ppm of total phosphorus. In other approaches, the phosphorus-containing additives provide about 200 to about 500 ppm of total phosphorus, about 200 to about 450 ppm of total phosphorus, about 200 to about 400 ppm of total phosphorus, about 200 to about 350 ppm of total phosphorus, about 200 to about 300 ppm of total phosphorus, or about 200 to about 250 ppm of total phosphorus. Even though higher levels of total phosphorus was previously thought necessary to achieve desired LSPI performance, the lubricants herein achieve good LSPI results with low levels of total phosphorus.

The one or more phosphorus-containing compounds may include metal containing phosphorus-containing compounds and/or ashless phosphorus-containing compounds.

Examples of suitable phosphorus-containing compound include, but are not limited to, thiophosphates, dithiophosphates, metal phosphates, metal thiophosphates, metal dithiophosphates, phosphates, phosphoric acid esters, phosphate esters, phosphites, phosphonates, phosphorus-containing carboxylic esters, ethers, or amides salts thereof, and mixtures thereof. In any of the above-described phosphorus-containing compounds, the compound may have about 5 to about 20 weight percent phosphorus, or about 5 to about 15 weight percent phosphorus, or about 8 to about 16 weight percent phosphorus, or about 6 to about 9 weight percent phosphorus.

One type of suitable phosphorus-containing compound is a metal dihydrocarbyl dithiophosphate compound, such as but not limited to, a zinc dihydrocarbyl dithiophosphate compound (i.e., ZDDP). When the phosphorus-containing compound is a metal thiophosphate or metal dithiophosphate, such as ZDDP, it may include between 5 to about 10 weight percent metal, about 6 to about 9 weight percent metal, about 8 to 18 weight percent sulfur, about 12 to about 18 weight percent sulfur, or about 8 to about 15 weight percent sulfur. Suitable metal dihydrocarbyl dithiophosphates may comprise dihydrocarbyl dithiophosphate metal salts wherein the metal may be an alkali metal, alkaline earth metal, aluminum, lead, tin, molybdenum, manganese, nickel, copper, titanium, zirconium, zinc, or combinations thereof, and preferably, the metal is zinc.

When the phosphorus-containing compound is a ZDDP, the alkyl groups on ZDDP may be derived from primary alcohols, secondary alcohols, phenols, and/or mixtures thereof. For example, all of the alkyl groups of ZDDP may be derived from a secondary alcohol such as methyl isobutyl carbinol, or from a mixture of secondary alcohols such as methyl isobutyl carbinol and isopropyl alcohol. In some cases, the alkyl groups of the ZDDP may be derived from a mixture of primary and secondary alcohols, such as 2-ethyl hexanol, isobutanol, and isopropanol. ZDDPs may include about 6 to about 10 weight percent phosphorus, about 6 to about 9 weight percent zinc, and about 12 to about 18 weight percent sulfur.

Examples of such ZDDPs include, but are not limited to: zinc O,O-di(Cp-4-alkyl)dithiophosphate; zinc (mixed O,O-bis(sec-butyl and isoctyl)) dithiophosphate; zinc-O,O-bis (branched and linear C<sub>3-8</sub>-alkyl)dithiophosphate; zinc O,O-bis(2-ethylhexyl) dithiophosphate; zinc O,O-bis(mixed isobutyl and pentyl)dithiophosphate; zinc mixed O,O-bis(1,3-dimethylbutyl and isopropyl)dithiophosphate; zinc O,O-diisooctyl dithiophosphate; zinc O,O-dibutyl dithiophosphate; zinc mixed O,O-bis(2-ethylhexyl and isobutyl and isopropyl)dithiophosphate; zinc O,O-bis(dodecylphenyl)dithiophosphate; zinc O,O-diisodecyl dithiophosphate; zinc O-(6-methylheptyl)-O-(1-methylpropyl)dithiophosphate; zinc O-(2-ethylhexyl)-O-(isobutyl)dithiophosphate; zinc O,O-diisopropyl dithiophosphate; zinc (mixed hexyl and isopropyl)dithiophosphate; zinc (mixed O-(2-ethylhexyl) and O-isopropyl) dithiophosphate; zinc O,O-diethyl dithiophosphate; zinc O,O-dipentyl dithiophosphate; zinc O-(2-methylbutyl)-O-(2-methylpropyl)dithiophosphate; and zinc O-(3-methylbutyl)-O-(2-methylpropyl)dithiophosphate.

Such phosphorus-containing compounds may have the formula:



wherein each R in Formula I, independently, contains from 1 to 18 carbon atoms, or 2 to 12 carbon atoms, or about 3 to 8 carbon atoms. For example, R may be ethyl, n-propyl, i-propyl, n-butyl, i-butyl, sec-butyl, amyl, n-hexyl, i-hexyl, n-octyl, decyl, dodecyl, octadecyl, 2-ethylhexyl, phenyl, butylphenyl, cyclohexyl, methylcyclopentyl, methylpentyl, propenyl, butenyl. The number of carbon atoms in each R group in the formula above will generally be about 3 or greater, about 4 or greater, about 6 or greater, or about 8 or greater. Each R group may average 3 to 8 carbons. The total number of carbon atoms in each R groups may be 5 to about 72, or 12 to about 32. In Formula I, A is a metal, such as aluminum, lead, tin, molybdenum, manganese, nickel, copper, titanium, zirconium, zinc, or combinations thereof.

15 When the phosphorus-containing compound has the structure shown in Formula I, the compound may have about 6 to about 9 weight percent phosphorus.

It is understood in the art that a more accurate representation of the sulfur-zinc coordination arrangement may be 20 represented by the symmetrical arrangement shown below the chemical structure of Formula I used herein is interchangeable with Formula I' shown below. It is also understood that the structures shown in Formulas I and I' may be 25 present as monomer, dimer, trimer, or oligomer (such as a tetramer).



Dihydrocarbyl dithiophosphate metal salts may be prepared in accordance with known techniques by first forming 30 a dihydrocarbyl dithiophosphoric acid (DDPA), usually by reaction of one or more alcohols or phenols with P<sub>2</sub>S<sub>5</sub> and then neutralizing the formed DDPA with a metal compound, such as zinc oxide. For example, DDPA may be made by reacting mixtures of primary and secondary alcohols with P<sub>2</sub>S<sub>5</sub>. In this case, the DDPA includes alkyl groups derived from both primary and secondary alcohols. Alternatively, 40 multiple DDPA can be prepared where the alkyl groups on one DDPA are derived entirely from secondary alcohols and the alkyl groups on another DDPA are derived entirely from primary alcohols. The DDPA are then blended together to form a mixture of DDPA having alkyl groups derived from both primary and secondary alcohols.

Another type of suitable phosphorus-containing compound for the lubricants herein may be an ashless (i.e., metal free) phosphorus-containing compound. In some embodiments, the ashless phosphorus-containing compound may be dialkyl dithiophosphate ester, amyl acid phosphate, diamyl acid phosphate, dibutyl hydrogen phosphonate, dimethyl octadecyl phosphonate, salts thereof, and mixtures thereof.

55 In some embodiments, an exemplary ashless phosphorus-containing compound may have the formula:



60 wherein R<sub>1</sub> is S or O; R<sub>2</sub> is —OR", —OH, or —R"; R<sub>3</sub> is —OR", —OH, or SR" C(O)OH; R<sub>4</sub> is —OR"; R" is C<sub>1</sub> to C<sub>3</sub>

branched or linear alkyl chain; and R" is a C1 to C18 hydrocarbyl chain of Formula II above.

In some embodiments, a phosphorus-containing compound of Formula II may have R<sub>1</sub> as S; R<sub>2</sub> as —OR"; R<sub>3</sub> as S R"COOH; R<sub>4</sub> as —OR"; R" as a C<sub>3</sub> branched alkyl chain; R" as C<sub>4</sub>. In another embodiment, a phosphorus-containing compound of Formula II may have R<sub>1</sub> as O; R<sub>2</sub> as —OH; R<sub>3</sub> as —OR" or —OH; R<sub>4</sub> as —OR"; R" as C<sub>5</sub>. In yet another embodiment, a phosphorus-containing compound of Formula II may have R<sub>1</sub> as O; R<sub>2</sub> as OR"; R<sub>3</sub> as H; R<sub>4</sub> as —OR"; R" as C<sub>4</sub>. In other embodiments, a phosphorus-containing compound of Formula II may have R<sub>1</sub> as O; R<sub>2</sub> as —R"; R<sub>3</sub> as —OCH<sub>3</sub> or —OH; R<sub>4</sub> as —OCH<sub>3</sub>; R" as Cis.

#### The Detergent System

The lubricating compositions herein may also include select detergent systems configured with certain relationships to work in combination with the low levels of phosphorus to achieve the improved LSPI. In some embodiments, the detergents herein contribute total base levels (TBN), measured pursuant to ASTM D2896, to the lubricating composition of at least about 1 mg KOH/g, of at least 2 mg KOH/g, of at least about 3 mg KOH/g, at least about 4 mg KOH/g, or at least about 5 mg KOH/g and up to about 15 mg KOH/g, up to about 12 mg KOH/g or less, up to about 10 mg KOH/g or less, or up to about 8 mg KOH/g. In embodiments, the detergent systems herein generally include one or more alkali or alkaline metal salts of sulfonates with minor amounts of, residual levels of, or preferably no other detergent additives such as phenates, calixarates, salixarates, salicylates, carboxylic acids, sulfu-  
5 rized derivatives thereof, or combinations thereof so long as the noted relationships are maintained herein. Preferably, the detergent systems herein are substantially free of phenate detergent additives (i.e., less than about 1 weight percent of phenate detergents, less than about 0.5 weight percent of phenate detergents, less than about 0.1 weight percent phenate detergents, less than about 0.05 weight percent phenate detergents, or no functional amounts of phenate detergents).

As discussed more below, the detergents herein preferably include one or more calcium-containing detergents, one or more optional magnesium-containing detergents, or combinations thereof. Preferably, the detergents are also substantially free of sodium-containing detergents (i.e., less than about 1 weight percent of sodium-containing detergents, less than about 0.5 weight percent of sodium-containing detergents, less than about 0.1 weight percent sodium-containing detergents, less than about 0.05 weight percent sodium-containing detergents, or no functional amounts of sodium-containing detergents).

In other approaches or embodiments, the detergent systems herein are also configured to maintain low levels of calcium content measured as calcium sulfated ash (Ca-SASH) pursuant to ASTM D874 or, more preferably, calculated based on the amount of metals in the lubricant. For example, sulfated ash (SASH) or calcium sulfated ash (Ca-SASH) may be calculated based on the total metallic elements that contribute to SASH in the lubricant composition adjusted by factors for each metallic type. The metals that contribute to SASH include (along with the adjustment factor) barium (1.7), boron (3.22), calcium (3.4), copper (1.252), lead (1.464), lithium (7.92), magnesium (4.95), manganese (1.291), molybdenum (1.5), potassium (2.33), sodium (3.09), and zinc (1.5). Specifically, the ppmw content of each of the metallic elements present in a lubricating oil composition that is considered to contribute to sulfated ash is multiplied by its corresponding factor above; then, the product for each metallic element/factor adjustment is

summed and the total is divided by 10,000 to calculate the weight percent of SASH in the lubricating compositions. Unless specified otherwise, all sulfated ash levels herein are calculated using this procedure.

In approaches, the detergents herein provide a calcium content that contributes no more than about 0.20 weight percent of Ca-SASH, no more than about 0.19 weight percent of Ca-SASH, or no more than about 0.18 weight of Ca-SASH. The lubricants may also have no more than about 1 weight percent of total sulfated ash content and, in other approaches, no more than about 0.8 weight percent of total sulfated ash content, or no more than about 0.7 weight percent of total sulfated ash content as measured pursuant to the calculations therein. In such embodiments, no more than 15 about 30 weight percent of the total sulfated ash content is provided by calcium sulfated ash, in other approaches, no more than about 28 percent, or no more than about 25 percent of the total sulfated ash content is contributed by calcium sulfated ash.

20 Suitable detergents and their methods of preparation are described in greater detail in numerous patent publications, including U.S. Pat. No. 7,732,390 and references cited therein, which are incorporated herein by reference. In some embodiments, the lubricant compositions herein may include about 0.1 to about 5 weight percent of any individual and/or total detergent additives, and in other approaches, about 0.15 to about 3 weight percent, and in yet other approaches, about 0.15 to 2.6 weight percent of individual and/or total detergent additives so long as the detergent additives meet the calcium, magnesium, SASH contents, sulfonate amounts, and/or other relationships noted herein.

Generally, suitable detergents in the systems herein, subject to the various relationships and metal contents noted above, may include linear or branched alkali or alkaline earth metal salts, such as calcium, sodium, or magnesium, of petroleum sulfonic acids and long chain mono- or di-alkylaryl sulfonic acids with the aryl group being benzyl, tolyl, and xylyl and/or various phenates or derivatives of phenates. Examples of suitable detergents include, subject 35 to the required amounts of sulfonate soap, low-based/neutral and overbased variations of the following detergents: calcium phenates, calcium sulfur containing phenates, calcium sulfonates, calcium calixarates, calcium salixarates, calcium salicylates, calcium carboxylic acids, calcium phosphorus acids, calcium mono- and/or di-thiophosphoric acids, calcium alkyl phenols, calcium sulfur coupled alkyl phenol compounds, calcium methylene bridged phenols, magnesium phenates, magnesium sulfur containing phenates, magnesium sulfonates, magnesium calixarates, magnesium salixarates, magnesium salicylates, magnesium carboxylic acids, magnesium phosphorus acids, magnesium mono- and/or di-thiophosphoric acids, magnesium alkyl phenols, magnesium sulfur coupled alkyl phenol compounds, magnesium methylene bridged phenols, sodium phenates, sodium sulfur containing phenates, sodium sulfonates, sodium calixarates, sodium salixarates, sodium salicylates, sodium carboxylic acids, sodium phosphorus acids, sodium mono- and/or di-thiophosphoric acids, sodium alkyl phenols, sodium sulfur coupled alkyl phenol compounds, or sodium methylene bridged phenols.

The detergent additives may be neutral, low-based, or overbased and, preferably, overbased calcium and magnesium detergents as needed to meet the minimum detergent TBN numbers as noted above. As understood, overbased detergent additives are well-known in the art and may be alkali or alkaline earth metal overbased detergent additives. Such detergent additives may be prepared by reacting a

metal oxide or metal hydroxide with a substrate and carbon dioxide gas. The substrate is typically an acid, for example, an acid such as an aliphatic substituted sulfonic acid, an aliphatic substituted carboxylic acid, or an aliphatic substituted phenol.

The term "overbased" relates to metal salts, such as metal salts of sulfonates, carboxylates, salicylates and/or phenates, wherein the amount of metal present exceeds the stoichiometric amount. Such salts may have a conversion level in excess of 100% (i.e., they may comprise more than 100% of the theoretical amount of metal needed to convert the acid to its "normal," "neutral" salt). The expression "metal ratio," often abbreviated as MR, is used to designate the ratio of total chemical equivalents of metal in the overbased salt to chemical equivalents of the metal in a neutral salt according to known chemical reactivity and stoichiometry. In a normal or neutral salt, the MR is one and in an overbased salt, MR, is greater than one. They are commonly referred to as overbased, hyperbased, or superbased salts and may be salts of organic sulfur acids, carboxylic acids, or phenols.

As used herein, the term "TBN" is used to denote the Total Base Number in mg KOH/g as measured by the method of ASTM D2896. The detergent may be neutral or overbased. For example, a neutral detergent may have a total base number (TBN) of up to about 200 mg KOH/gram. In another example, an overbased detergent of the lubricating oil compositions herein may have a total base number (TBN) of about 200 mg KOH/gram or greater, or about 250 mg KOH/gram or greater, or about 350 mg KOH/gram or greater, or about 375 mg KOH/gram or greater, or about 400 mg KOH/gram or greater. The overbased detergent may have a metal to substrate ratio of from 1.1:1 or less, or from 2:1 or less, or from 4:1 or less, or from 5:1 or less, or from 7:1 or less, or from 10:1 or less, or from 12:1 or less, or from 15:1 or less, or from 20:1 or less.

Examples of suitable overbased detergents (so long as the calcium, magnesium, SASH, TBN, and other relationships noted herein are satisfied) include, but are not limited to, overbased calcium phenates, overbased calcium sulfur containing phenates, overbased calcium sulfonates, overbased calcium calixarates, overbased calcium salixarates, overbased calcium salicylates, overbased calcium carboxylic acids, overbased calcium phosphorus acids, overbased calcium mono- and/or di-thiophosphoric acids, overbased calcium alkyl phenols, overbased calcium sulfur coupled alkyl phenol compounds, overbased calcium methylene bridged phenols, overbased magnesium phenates, overbased magnesium sulfur containing phenates, overbased magnesium sulfonates, overbased magnesium calixarates, overbased magnesium salixarates, overbased magnesium salicylates, overbased magnesium carboxylic acids, overbased magnesium phosphorus acids, overbased magnesium mono- and/or di-thiophosphoric acids, overbased magnesium alkyl phenols, overbased magnesium sulfur coupled alkyl phenol compounds, or overbased magnesium methylene bridged phenols.

Optionally, the detergents herein may include low-based or neutral detergent so long as the other fluid relationships described herein are satisfied. When an optional low-based or neutral detergent is incorporated into the detergent system, it generally has a TBN of up to 175 mg KOH/g, up to 150 mg KOH/g, up to 100 mg KOH/g, or up to 50 mg KOH/g. The low-based/neutral detergent may include a calcium or magnesium-containing detergent. Examples of suitable low-based/neutral detergent (again, so long as the calcium, TBN, SASH, and other relationships noted herein are satisfied) include, but are not limited to, calcium

sulfonates, calcium phenates, calcium salicylates, magnesium sulfonates, magnesium phenates, and/or magnesium salicylates.

In some embodiments, the detergent used in the lubricants herein include at least an overbased calcium sulfonate and/or an overbased magnesium sulfonate with each having a total base number of 150 to 450 and, in other approaches, about 200 to about 400, or about 200 to about 350. The above described TBN values reflect those of finished detergent components that have been diluted in a base oil. In other embodiments, the TBN of the detergents herein may reflect a neat (i.e., non-diluted or oil-free) version of the detergent component. For example, the fluids herein may include overbased calcium as a neat additive having a TBN of about 300 to about 450, and in other approaches, about 380 to about 420, and/or overbased magnesium sulfonate as a neat additive having a TBN of about 500 to about 700, and in other approaches, about 600 to about 700.

In some embodiments, the detergent systems herein have select levels of the calcium-based detergents to control the amount of calcium sulfated ash content (Ca-SASH) in the lubricants so that the lubricants achieve a selected weight ratio of the phosphorus content to the calcium sulfated ash content, which has been discovered to aid in improving the LSPI performance when using low levels of total phosphorus. For instance, and in embodiments herein, the lubricants have a weight ratio of the phosphorus content to the calcium sulfated ash content (Ca-SASH) of at least about 0.1, and in other approaches, about 0.1 to about 0.3. As used herein, the weight ratio of the phosphorus content to the calcium sulfated ash content is the weight percent phosphorus in the lubricant divided by the weight percent of calcium sulfated ash (calculated as described herein) in the lubricant as shown below in the Examples.

#### 35 Silicon-Containing Compounds

In approaches or embodiments, the lubricating compositions herein may also include one or more optional silicon-containing compounds. For example, the compositions may include one or more organosilane compounds, fluorosilicone compounds, polydimethyl siloxane compounds, phenyl-methyl polysiloxane compounds, linear siloxane compounds, cyclic siloxane compounds, branched siloxane compounds, silicone polymers and copolymers, organo-silicone copolymers, and mixtures thereof. In some approaches, such silicon-containing compounds may have a kinematic viscosity at 25° C. of greater than about 20,000 cSt, and, in some approaches, may be about 40,000 to about 80,000 cSt at 25° C.

For example, suitable organosilane compounds may include, but are not limited to, hydrocarbyl silyl ether compounds such as those having C6 to C20 hydrocarbyl chains. In one approach, an exemplary hydrocarbyl silyl ether compound may be a tri-alkoxy (hydrocarbyl) silane, such as a C10-C20 hydrocarbyl trimethoxy silane or more preferably, a C14-C20 hydrocarbyl trimethoxy silane, and most preferably hexadecyl trimethoxy silane. In other approaches, suitable silicon-containing compounds may be polysiloxane compounds and may include one or more silicone-based oils or one or more polydimethylsiloxane polymers. In yet other approaches, the silicon-containing compounds may be, but not limited to, hexadecyltrimethoxysilane, octyltriethoxysilane, nonyltriethoxysilane, n-decyltriethoxysilane, undecyl-triethoxysilane, and tetradecyltriethoxysilane. Preferably, the silicon-containing compounds may be silicone oil or polydimethylsiloxane polymers.

In other embodiments, suitable organosilanes may include one organic substituent and three hydrolysable substituents.

## 11

In yet other embodiments, exemplary organosilanes may include, but are not limited to, the following compounds: [2-(3-cyclohexenyl) ethyl]trimethoxysilane, trimethoxy(7-octen-1-yl) silane, isoctyl trimethoxy-silane, N-(3-triethoxy-silylpropyl) methoxyethoxyethoxyethyl carbamate, N-(3-triethoxysilylpropyl) methoxy-ethoxyethoxyethyl carbamate, 3-(methacryloyloxy)propyltrimethoxysilane, allyl trimethoxysilane, 3-acryloxypropyltrimethoxysilane, 3-(methacryloyloxy) propyltrimethoxysilane, 3-(methacryloyloxy) propylmethyldimethoxysilane, 3-(acryloyloxypropyl) methyl-dimethoxysilane, 9-3-(methacryloyloxy)propyltrimethylethoxysilane, 3-(methacryloyloxy) propyltrimethoxysilane, vinyltrimethylethoxysilane, phenyltrimethoxysilane, n-octyltrimethoxysilane, dodecyltrimethoxysilane, isoctyltrimethoxysilane, octadecyltrimethoxysilane, propyltrimethoxysilane, hexyltrimethoxysilane, vinylmethyl-diacetoxysilane, vinylmethylidethoxysilane, vinyltriacetoxysilane, vinyltriethoxysilane, vinyltriisopropoxysilane, vinyltrimethoxysilane, vinyltriphenoxysilane, vinyltri-t-butoxysilane, vinyltris-isobutoxysilane, vinyltrisopropen-oxysilane, vinyltris(2-methoxyethoxy) silane, styrelithyltrimethoxysilane, mercaptopropyl-trimethoxysilane, 3-glycidoxypropyltrimethoxysilane, heptamethyl(2-ltris(2-methoxyethoxy) silyl)hexyltrisiloxane (as described in US 2003/0220204) poly dimethylsiloxane, arylsilanes, including, for instance, substituted and unsubstituted arylsilanes, alkylsilanes, including, substituted and unsubstituted alkyl silanes, including, methoxy and hydroxy substituted alkyl silanes, and/or combinations of two or more of the foregoing compounds.

In approaches or embodiments, the silicon-containing compound is present in an amount sufficient to provide about 3 ppm to about 20 ppm of silicon to the lubricating oil composition, in other approaches, about 4 ppm to about 18 ppm of silicon, about 5 ppm to about 15 ppm of silicon, or about 7 ppm to about 15 ppm of silicon to the lubricating oil composition.

In some embodiments, the lubricating compositions herein may also have a unique weight ratio of the calcium sulfated ash content to the silicon content that may also aid in providing the improved LSPI performance when using the low levels of total phosphorus herein. For instance, and in some embodiments, the lubricants herein may have a weight ratio of the calcium sulfated ash content to the silicon content of no more than 250:1, and in other approaches, about 100:1 to about 250:1 to aid in achieving the improvements in LSPI noted herein with the low levels of total phosphorus. As used herein, the weight ratio of the calcium sulfated ash content to the silicon content is the weight percent of calcium sulfated ash in the lubricant divided by the weight percent of the silicon content in the lubricant as shown below in the Examples.

## Dispersants

The lubricating compositions herein may also include one or more optional dispersants. Dispersants are often known as ashless-type dispersants because, prior to mixing in a lubricating composition, they do not contain ash-forming metals and they do not normally contribute any ash when added to a lubricant. Ashless type dispersants are characterized by a polar group attached to a relatively high molecular weight hydrocarbon chain. Typical ashless dispersants include N-substituted long chain alkenyl succinimides. Examples of N-substituted long chain alkenyl succinimides include polyisobutylene succinimide with the number average molecular weight of the polyisobutylene substituent being in the range about 350 to about 50,000, or to about 5,000, or to about 3,000, or to about 2,000, or to about 1,500 as measured by

## 12

GPC. Succinimide dispersants and their preparation are disclosed, for instance in U.S. Pat. No. 7,897,696 or U.S. Pat. No. 4,234,435, which are incorporated herein by reference. The alkenyl substituent may be prepared from polymerizable monomers containing about 2 to about 16, or about 2 to about 8, or about 2 to about 6 carbon atoms. Succinimide dispersants are typically the imide formed from a polyamine, typically a poly(ethyleneamine).

In approaches, preferred amines for the dispersants may be selected from polyamines and hydroxylamines. Examples of polyamines that may be used include, but are not limited to, diethylene triamine (DETA), triethylene tetramine (TETA), tetraethylene pentamine (TEPA), and higher homologues such as pentaethylene hexamine (PEHA), and the like. In some approaches, a so-called heavy polyamine may be used, which is a mixture of polyalkylene-polyamines comprising small amounts of lower polyamine oligomers such as TEPA and PEHA (pentaethylene hexamine) but primarily oligomers with 6 or more nitrogen atoms, 2 or more primary amines per molecule, and more extensive branching than conventional polyamine mixtures. A heavy polyamine preferably includes polyamine oligomers containing 7 or more nitrogen atoms per molecule and with 2 or more primary amines per molecule.

In some embodiments, polyisobutylene (PIB), when included, is a preferred reactant to form the dispersants and may have greater than 50 mol %, greater than 60 mol %, greater than 70 mol %, greater than 80 mol %, or greater than 90 mol % content of terminal double bonds. Such PIB is also referred to as highly reactive PIB ("HR-PIB"). HR-PIB having a number average molecular weight ranging from about 800 to about 5000, as determined by GPC, is suitable for use in embodiments of the present disclosure. Conventional PIB typically has less than 50 mol %, less than 40 mol %, less than 30 mol %, less than 20 mol %, or less than 10 mol % content of terminal double bonds.

An HR-PIB having a number average molecular weight ranging from about 900 to about 3,000 may be suitable, as determined by GPC. Such HR-PIB is commercially available, or can be synthesized by the polymerization of isobutene in the presence of a non-chlorinated catalyst such as boron trifluoride, as described in U.S. Pat. No. 4,152,499 and/or U.S. Pat. No. 5,739,355. When used in the aforementioned thermal ene reaction, HR-PIB may lead to higher conversion rates in the reaction, as well as lower amounts of sediment formation, due to increased reactivity. A suitable method is described in U.S. Pat. No. 7,897,696. In one embodiment, the present disclosure further comprises at least one dispersant derived from polyisobutylene succinic anhydride ("PIBSA"). The PIBSA may have an average of between about 1.0 and about 2.0 succinic acid moieties per polymer.

In some approaches, the dispersants in the lubricants herein may optionally be post-treated by conventional methods by a reaction with any of a variety of agents. Suitable post treat agents include boron, urea, thiourea, dimercaptothiadiazoles, carbon disulfide, aldehydes, ketones, carboxylic acids, hydrocarbon-substituted succinic anhydrides, maleic anhydride, nitriles, epoxides, carbonates, cyclic carbonates, hindered phenolic esters, and phosphorus compounds. (See, e.g., U.S. Pat. Nos. 7,645,726; 7,214,649; 8,048,831; and 5,241,003, which are all incorporated herein by reference in their entireties.)

The boron compound used as a post-treating reagent can be selected from boron oxide, boron halides, boron acids and esters of boron acids in an amount to provide from about 0.1 atomic proportion of boron for each mole of the nitrogen

## 13

composition to about 20 atomic proportions of boron for each atomic proportion of nitrogen used. The dispersant post-treated with boron may contain from about 0.05 weight percent to about 2.0 weight percent, or in other approaches, about 0.05 weight percent to about 0.9 weight percent boron, based on the total weight of the borated dispersant.

In other approaches, carboxylic acid may also be used as a post-treating reagent and can be saturated or unsaturated mono-, di-, or poly-carboxylic acid. Examples of carboxylic acids include, but are not limited to, maleic acid, fumaric acid, succinic acid, and naphthalic diacid (e.g., 1,8-naphthalic diacid). Anhydrides can also be used as a post-treating reagent and can be selected from the group consisting of mono-unsaturated anhydride (e.g., maleic anhydride), alkyl or alkylene-substituted cyclic anhydrides (e.g., succinic anhydride or glutamic anhydride), and aromatic carboxylic anhydrides (including naphthalic anhydride, e.g., 1,8-naphthalic anhydride).

In one embodiment, the process of post-treating the dispersant includes first forming the succinimide product, as described above, and then further reacting the succinimide product with the post treating agent, such as a boron compound, such as boric acid. In some cases, the dispersants herein may be post-treated with more than one post-treatment agents. For example, the dispersant may be post-treated with a boron compound, such as boric acid, and also an anhydride, such as maleic anhydride and/or 1,8-naphthalic anhydride.

The dispersant can be used in an amount sufficient to provide up to about 20 weight percent of the lubricating composition and wherein one or more of the dispersants are post treated to provide at least about 40 ppm of boron and up to 500 ppm of boron to the lubricating composition. In other approaches, the dispersant may be used in the lubricating composition in amounts from about 0.1 weight percent to about 15 weight percent, or about 0.1 weight percent to about 10 weight percent, about 0.1 weight percent to 8 weight percent, or about 1 weight percent to about 10 weight percent, or about 1 weight percent to about 8 weight percent, or about 1 weight percent to about 6 weight percent, based upon the final weight of the lubricating oil composition. Dispersants may provide at least about 400 ppm nitrogen and up to about 1,500 ppm nitrogen.

#### Base Oil or Base Oil Blend:

The base oil used in the lubricating compositions herein may be oils of lubricating viscosity and selected from any of the base oils in API Groups I to V as specified in the American Petroleum Institute (API) Base Oil Interchangeability Guidelines. In one approach, the base oil of the lubricating compositions herein may be a blend of API Group II base oils combined with API Group III base oils. Surprisingly, when the fluid elemental relationships noted above are followed, even the lower quality base oils may be used in the lubricants herein. The five base oil groups are generally set forth in Table 1 below:

TABLE 1

| Base oil Category | Sulfur (%)                                          | Saturates (%) | Viscosity Index |
|-------------------|-----------------------------------------------------|---------------|-----------------|
| Group I           | >0.03                                               | and/or        | <90 80 to 120   |
| Group II          | ≤0.03                                               | and           | ≥90 80 to 120   |
| Group III         | ≤0.03                                               | and           | ≥90 ≥120        |
| Group IV          | All polyalphaolefins (PAOs)                         |               |                 |
| Group V           | All others not included in Groups I, II, III, or IV |               |                 |

## 14

Groups I, II, and III are mineral oil process stocks. Group IV base oils contain true synthetic molecular species, which are produced by polymerization of olefinically unsaturated hydrocarbons. Many Group V base oils are also true synthetic products and may include diesters, polyol esters, polyalkylene glycols, alkylated aromatics, polyphosphate esters, polyvinyl ethers, and/or polyphenyl ethers, and the like, but may also be naturally occurring oils, such as vegetable oils. It should be noted that although Group III base oils are derived from mineral oil, the rigorous processing that these fluids undergo causes their physical properties to be very similar to some true synthetics, such as PAOs. Therefore, oils derived from Group III base oils may be referred to as synthetic fluids in the industry. Group II+ may comprise high viscosity index Group II.

The base oil blend used in the disclosed lubricating oil composition may be a mineral oil, animal oil, vegetable oil, synthetic oil, synthetic oil blends, or mixtures thereof. Suitable oils may be derived from hydrocracking, hydrogeneration, hydrofinishing, unrefined, refined, and re-refined oils, and mixtures thereof.

Unrefined oils are those derived from a natural, mineral, or synthetic source without or with little further purification treatment. Refined oils are similar to the unrefined oils except that they have been treated in one or more purification steps, which may result in the improvement of one or more properties. Examples of suitable purification techniques are solvent extraction, secondary distillation, acid or base extraction, filtration, percolation, and the like. Oils refined to the quality of an edible may or may not be useful. Edible oils may also be called white oils. In some embodiments, lubricating oil compositions are free of edible or white oils.

Re-refined oils are also known as reclaimed or reprocessed oils. These oils are obtained similarly to refined oils using the same or similar processes. Often these oils are additionally processed by techniques directed to removal of spent additives and oil breakdown products.

Mineral oils may include oils obtained by drilling or from plants and animals or any mixtures thereof. For example, such oils may include, but are not limited to, castor oil, lard oil, olive oil, peanut oil, corn oil, soybean oil, and linseed oil, as well as mineral lubricating oils, such as liquid petroleum oils and solvent-treated or acid-treated mineral lubricating oils of the paraffinic, naphthenic or mixed paraffinic-naphthenic types. Such oils may be partially or fully hydrogenated, if desired. Oils derived from coal or shale may also be useful.

Useful synthetic lubricating oils may include hydrocarbon oils such as polymerized, oligomerized, or interpolymerized olefins (e.g., polybutylenes, polypropylenes, propyleneisobutylene copolymers); poly(1-hexenes), poly(1-octenes), trimers or oligomers of 1-decene, e.g., poly(1-decenes), such materials being often referred to as  $\alpha$ -olefins, and mixtures thereof; alkyl-benzenes (e.g. dodecylbenzenes, tetradecylbenzenes, dinonylbenzenes, di-(2-ethylhexyl)-benzenes); polyphenyls (e.g., biphenyls, terphenyls, alkylated polyphenyls); diphenyl alkanes, alkylated diphenyl alkanes, alkylated diphenyl ethers and alkylated diphenyl sulfides and the derivatives, analogs and homologs thereof or mixtures thereof. Polyalphaolefins are typically hydrogenated materials.

Other synthetic lubricating oils include polyol esters, diesters, liquid esters of phosphorus-containing acids (e.g., tricresyl phosphate, trioctyl phosphate, and the diethyl ester of decane phosphonic acid), or polymeric tetrahydrofurans. Synthetic oils may be produced by Fischer-Tropsch reac-

tions and typically may be hydroisomerized Fischer-Tropsch hydrocarbons or waxes. In one embodiment oils may be prepared by a Fischer-Tropsch gas-to-liquid synthetic procedure as well as other gas-to-liquid oils.

The major amount of base oil included in a lubricating composition may be selected from the group consisting of Group I, Group II, a Group III, a Group IV, a Group V, and a combination of two or more of the foregoing, and wherein the major amount of base oil is other than base oils that arise from provision of additive components or viscosity index improvers in the composition. In another embodiment, the major amount of base oil included in a lubricating composition may be selected from the group consisting of Group II, a Group III, a Group IV, a Group V, and a combination of two or more of the foregoing, and wherein the major amount of base oil is other than base oils that arise from provision of additive components or viscosity index improvers in the composition.

The amount of the oil of lubricating viscosity present may be the balance remaining after subtracting from 100 wt. % the sum of the amount of the performance additives inclusive of viscosity index improver(s) and/or pour point depressant(s) and/or other top treat additives. For example, the oil of lubricating viscosity that may be present in a finished fluid may be a major amount, such as greater than about 50 wt. %, greater than about 60 wt. %, greater than about 70 wt. %, greater than about 80 wt. %, greater than about 85 wt. %, or greater than about 90 wt. %.

The base oil systems herein, in some approaches or embodiments, include one or more of a Group I to Group V base oils and may have a KV100 of about 2 to about 20 cSt, in other approaches, about 2 to about 10 cSt, about 2.5 to about 6 cSt, in yet other approaches, about 2.5 to about 3.5 cSt, and in other approaches about 2.5 to about 4.5 cSt. (ASTM D445)

As used herein, the terms "oil composition," "lubrication composition," "lubricating oil composition," "lubricating oil," "lubricant composition," "fully formulated lubricant composition," "lubricant," and "lubricating and cooling fluid" are considered synonymous, fully interchangeable terminology referring to the finished lubrication product comprising a major amount of a base oil component plus minor amounts of the detergents and the other optional components.

#### Optional Additives:

The lubricating oil compositions herein may also include a number of optional additives combined with the detergent systems, sulfurized additives, and boronated detergents as needed to meet performance standards. Those optional additives are described in the following paragraphs.

**Other Dispersants:** The lubricating oil composition may optionally include one or more other dispersants or mixtures thereof. Dispersants are often known as ashless-type dispersants because, prior to mixing in a lubricating oil composition, they do not contain ash-forming metals and they do not normally contribute any ash when added to a lubricant. Ashless type dispersants are characterized by a polar group attached to a relatively high molecular weight hydrocarbon chain. Typical ashless dispersants include N-substituted long chain alkenyl succinimides. Examples of N-substituted long chain alkenyl succinimides include polyisobutylene succinimide with the number average molecular weight of the polyisobutylene substituent being in the range about 350 to about 50,000, or to about 5,000, or to about 3,000, as measured by GPC. Succinimide dispersants and their preparation are disclosed, for instance in U.S. Pat. No. 7,897,696 or U.S. Pat. No. 4,234,435. The alkenyl substituent may be

prepared from polymerizable monomers containing about 2 to about 16, or about 2 to about 8, or about 2 to about 6 carbon atoms. Succinimide dispersants are typically the imide formed from a polyamine, typically a poly(ethyl-5 eneamine).

Preferred amines are selected from polyamines and hydroxylamines. Examples of polyamines that may be used include, but are not limited to, diethylene triamine (DETA), triethylene tetramine (TETA), tetraethylene pentamine 10 (TEPA), and higher homologues such as pentaethylene hexamine (PEHA), and the like.

A suitable heavy polyamine is a mixture of polyalkylene-polyamines comprising small amounts of lower polyamine oligomers such as TEPA and PEHA (pentaethylene hexamine) but primarily oligomers with 6 or more nitrogen atoms, 2 or more primary amines per molecule, and more extensive branching than conventional polyamine mixtures. A heavy polyamine preferably includes polyamine oligomers containing 7 or more nitrogen atoms per molecule and with 2 or more primary amines per molecule. The heavy polyamine comprises more than 28 wt. % (e.g. >32 wt. %) total nitrogen and an equivalent weight of primary amine groups of 120-160 grams per equivalent.

In some approaches, suitable polyamines are commonly known as PAM and contain a mixture of ethylene amines where TEPA and pentaethylene hexamine (PEHA) are the major part of the polyamine, usually less than about 80%.

Typically, PAM has 8.7-8.9 milliequivalents of primary amine per gram (an equivalent weight of 115 to 112 grams per equivalent of primary amine) and a total nitrogen content of about 33-34 wt. %. Heavier cuts of PAM oligomers with practically no TEPA and only very small amounts of PEHA but containing primarily oligomers with more than 6 nitrogen atoms and more extensive branching, may produce dispersants with improved dispersancy.

In an embodiment the present disclosure further comprises at least one polyisobutylene succinimide dispersant derived from polyisobutylene with a number average molecular weight in the range about 350 to about 50,000, or 40 to about 5000, or to about 3000, as determined by GPC. The polyisobutylene succinimide may be used alone or in combination with other dispersants.

In some embodiments, polyisobutylene, when included, may have greater than 50 mol %, greater than 60 mol %, 45 greater than 70 mol %, greater than 80 mol %, or greater than 90 mol % content of terminal double bonds. Such PIB is also referred to as highly reactive PIB ("HR-PIB"). HR-PIB having a number average molecular weight ranging from about 800 to about 5000, as determined by GPC, is suitable 50 for use in embodiments of the present disclosure. Conventional PIB typically has less than 50 mol %, less than 40 mol %, less than 30 mol %, less than 20 mol %, or less than 10 mol % content of terminal double bonds.

An HR-PIB having a number average molecular weight 55 ranging from about 900 to about 3000 may be suitable, as determined by GPC. Such HR-PIB is commercially available, or can be synthesized by the polymerization of isobutene in the presence of a non-chlorinated catalyst such as boron trifluoride, as described in U.S. Pat. No. 4,152,499 60 to Boerzel, et al. and U.S. Pat. No. 5,739,355 to Gateau, et al. When used in the aforementioned thermal ene reaction, HR-PIB may lead to higher conversion rates in the reaction, as well as lower amounts of sediment formation, due to increased reactivity. A suitable method is described in U.S. 65 Pat. No. 7,897,696.

In one embodiment, the present disclosure further comprises at least one dispersant derived from polyisobutylene

succinic anhydride ("PIBSA"). The PIBSA may have an average of between about 1.0 and about 2.0 succinic acid moieties per polymer.

The % actives of the alkenyl or alkyl succinic anhydride can be determined using a chromatographic technique. This method is described in column 5 and 6 in U.S. Pat. No. 5,334,321.

The percent conversion of the polyolefin is calculated from the % actives using the equation in column 5 and 6 in U.S. Pat. No. 5,334,321.

Unless stated otherwise, all percentages are in weight percent and all molecular weights are number average molecular weights determined by gel permeation chromatography (GPC) using commercially available polystyrene standards (with a number average molecular weight of 180 to about 18,000 as the calibration reference).

In one embodiment, the dispersant may be derived from a polyalphaolefin (PAO) succinic anhydride. In one embodiment, the dispersant may be derived from olefin maleic anhydride copolymer. As an example, the dispersant may be described as a poly-PIBSA. In an embodiment, the dispersant may be derived from an anhydride which is grafted to an ethylene-propylene copolymer.

A suitable class of nitrogen-containing dispersants may be derived from olefin copolymers (OCP), more specifically, ethylene-propylene dispersants which may be grafted with maleic anhydride. A more complete list of nitrogen-containing compounds that can be reacted with the functionalized OCP are described in U.S. Pat. Nos. 7,485,603; 7,786,057; 7,253,231; 6,107,257; and 5,075,383; and/or are commercially available.

One class of suitable dispersants may also be Mannich bases. Mannich bases are materials that are formed by the condensation of a higher molecular weight, alkyl substituted phenol, a polyalkylene polyamine, and an aldehyde such as formaldehyde. Mannich bases are described in more detail in U.S. Pat. No. 3,634,515.

A suitable class of dispersants may also be high molecular weight esters or half ester amides. A suitable dispersant may also be post-treated by conventional methods by a reaction with any of a variety of agents. Among these are boron, urea, thiourea, dimercaptothiadiazoles, carbon disulfide, aldehydes, ketones, carboxylic acids, hydrocarbon-substituted succinic anhydrides, maleic anhydride, nitriles, epoxides, carbonates, cyclic carbonates, hindered phenolic esters, and phosphorus compounds. U.S. Pat. Nos. 7,645,726; 7,214,649; and 8,048,831 are incorporated herein by reference in their entireties.

In addition to the carbonate and boric acids post-treatments both the compounds may be post-treated, or further post-treatment, with a variety of post-treatments designed to improve or impart different properties. Such post-treatments include those summarized in columns 27-29 of U.S. Pat. No. 5,241,003, hereby incorporated by reference. Such treatments include, treatment with: Inorganic phosphorous acids or anhydrides (e.g., U.S. Pat. Nos. 3,403,102 and 4,648,980); Organic phosphorous compounds (e.g., U.S. Pat. No. 3,502,677); Phosphorous pentasulfides; Boron compounds as already noted above (e.g., U.S. Pat. Nos. 3,178,663 and 4,652,387); Carboxylic acid, polycarboxylic acids, anhydrides and/or acid halides (e.g., U.S. Pat. Nos. 3,708,522 and 4,948,386); Epoxides polyepoxides or thioepoxides (e.g., U.S. Pat. Nos. 3,859,318 and 5,026,495); Aldehyde or ketone (e.g., U.S. Pat. No. 3,458,530); Carbon disulfide (e.g., U.S. Pat. No. 3,256,185); Glycidol (e.g., U.S. Pat. No. 4,617,137); Urea, thiourea or guanidine (e.g., U.S. Pat. Nos. 3,312,619; 3,865,813; and British Patent GB 1,065,595);

Organic sulfonic acid (e.g., U.S. Pat. No. 3,189,544 and British Patent GB 2,140,811); Alkenyl cyanide (e.g., U.S. Pat. Nos. 3,278,550 and 3,366,569); Diketene (e.g., U.S. Pat. No. 3,546,243); A diisocyanate (e.g., U.S. Pat. No. 3,573,205); Alkane sulfone (e.g., U.S. Pat. No. 3,749,695); 1,3-Dicarbonyl Compound (e.g., U.S. Pat. No. 4,579,675); Sulfate of alkoxylated alcohol or phenol (e.g., U.S. Pat. No. 3,954,639); Cyclic lactone (e.g., U.S. Pat. Nos. 4,617,138; 4,645,515; 4,668,246; 4,963,275; and 4,971,711); Cyclic 10 carbonate or thiocarbonate linear monocarbonate or polycarbonate, or chloroformate (e.g., U.S. Pat. Nos. 4,612,132; 4,647,390; 4,648,886; 4,670,170); Nitrogen-containing carboxylic acid (e.g., U.S. Pat. No. 4,971,598 and British Patent GB 2,140,811); Hydroxy-protected chlorodicarbonyloxy 15 compound (e.g., U.S. Pat. No. 4,614,522); Lactam, thiolactam, thiolactone or dithiolactone (e.g., U.S. Pat. Nos. 4,614,603 and 4,666,460); Cyclic carbonate or thiocarbonate, linear monocarbonate or polycarbonate, or chloroformate (e.g., U.S. Pat. Nos. 4,612,132; 4,647,390; 4,646,860; 20 and 4,670,170); Nitrogen-containing carboxylic acid (e.g., U.S. Pat. No. 4,971,598 and British Patent GB 2,440,811); Hydroxy-protected chlorodicarbonyloxy compound (e.g., U.S. Pat. No. 4,614,522); Lactam, thiolactam, thiolactone or 25 dithiolactone (e.g., U.S. Pat. Nos. 4,614,603, and 4,666,460); Cyclic carbamate, cyclic thiocarbamate or cyclic dithiocarbamate (e.g., U.S. Pat. Nos. 4,663,062 and 4,666,459); Hydroxyaliphatic carboxylic acid (e.g., U.S. Pat. Nos. 4,482,464; 4,521,318; 4,713,189); Oxidizing agent (e.g., U.S. Pat. No. 4,379,064); Combination of phosphorus pentasulfide 30 and a polyalkylene polyamine (e.g., U.S. Pat. No. 3,185,647); Combination of carboxylic acid or an aldehyde or ketone and sulfur or sulfur chloride (e.g., U.S. Pat. Nos. 3,390,086; 3,470,098); Combination of a hydrazine and carbon disulfide (e.g., U.S. Pat. No. 3,519,564); Combination 35 of an aldehyde and a phenol (e.g., U.S. Pat. Nos. 3,649,229; 5,030,249; 5,039,307); Combination of an aldehyde and an O-diester of dithiophosphoric acid (e.g., U.S. Pat. No. 3,865,740); Combination of a hydroxyaliphatic carboxylic acid and a boric acid (e.g., U.S. Pat. No. 4,554,086); Combination 40 of a hydroxyaliphatic carboxylic acid, then formaldehyde and a phenol (e.g., U.S. Pat. No. 4,636,322); Combination of a hydroxyaliphatic carboxylic acid and then an aliphatic dicarboxylic acid (e.g., U.S. Pat. No. 4,663,064); Combination of formaldehyde and a phenol and then glycolic acid (e.g., U.S. Pat. No. 4,699,724); Combination of a 45 hydroxyaliphatic carboxylic acid or oxalic acid and then a diisocyanate (e.g., U.S. Pat. No. 4,713,191); Combination of inorganic acid or anhydride of phosphorus or a partial or total sulfur analog thereof and a boron compound (e.g., U.S. Pat. No. 4,857,214); Combination of an organic diacid then an unsaturated fatty acid and then a nitroaromatic amine 50 optionally followed by a boron compound and then a glycolating agent (e.g., U.S. Pat. No. 4,973,412); Combination of an aldehyde and a triazole (e.g., U.S. Pat. No. 4,963,278); Combination of an aldehyde and a triazole then a boron compound (e.g., U.S. Pat. No. 4,981,492); Combination 55 of cyclic lactone and a boron compound (e.g., U.S. Pat. Nos. 4,963,275 and 4,971,711). The above-mentioned patents are herein incorporated in their entireties.

60 The TBN of a suitable dispersant may be from about 10 to about 65 mg KOH/g dispersant, on an oil-free basis, which is comparable to about 5 to about 30 TBN if measured on a dispersant sample containing about 50% diluent oil. TBN is measured by the method of ASTM D2896.

65 In yet other embodiments, the optional dispersant additive may be a hydrocarbyl substituted succinamide or succinimide dispersant. In approaches, the hydrocarbyl substituted

succinamide or succinimide dispersant may be derived from a hydrocarbyl substituted acylating agent reacted with a polyalkylene polyamine and wherein the hydrocarbyl substituent of the succinamide or the succinimide dispersant is a linear or branched hydrocarbyl group having a number average molecular weight of about 250 to about 5,000 as measured by GPC using polystyrene as a calibration reference.

In some approaches, the polyalkylene polyamine used to form the dispersant has the Formula



wherein each R and R', independently, is a divalent C1 to C6 alkylene linker, each R<sub>1</sub> and R<sub>2</sub>, independently, is hydrogen, a C1 to C6 alkyl group, or together with the nitrogen atom to which they are attached form a 5- or 6-membered ring optionally fused with one or more aromatic or non-aromatic rings, and n is an integer from 0 to 8. In other approaches, the polyalkylene polyamine is selected from the group consisting of a mixture of polyethylene polyamines having an average of 5 to 7 nitrogen atoms, triethylenetetramine, tetraethylenepentamine, and combinations thereof.

The dispersant, if present, can be used in an amount sufficient to provide up to about 20 wt. %, based upon the final weight of the lubricating oil composition. Another amount of the dispersant that can be used may be about 0.1 wt. % to about 15 wt. %, or about 0.1 wt. % to about 10 wt. %, about 0.1 to 8 wt. %, or about 1 wt. % to about 10 wt. %, or about 1 wt. % to about 8 wt. %, or about 1 wt. % to about 6 wt. %, based upon the final weight of the lubricating oil composition. In some embodiments, the lubricating oil composition utilizes a mixed dispersant system. A single type or a mixture of two or more types of dispersants in any desired ratio may be used.

**Antioxidants:** The lubricating oil compositions herein also may optionally contain one or more antioxidants. Antioxidant compounds are known and include for example, phenates, phenate sulfides, sulfurized olefins, phosphosulfurized terpenes, sulfurized esters, aromatic amines, alkylated diphenylamines (e.g., nonyl diphenylamine, di-nonyl diphenylamine, octyl diphenylamine, di-octyl diphenylamine), phenyl-alpha-naphthylamines, alkylated phenyl-alpha-naphthylamines, hindered non-aromatic amines, phenols, hindered phenols, oil-soluble molybdenum compounds, macromolecular antioxidants, or mixtures thereof. Antioxidant compounds may be used alone or in combination.

The hindered phenol antioxidant may contain a secondary butyl and/or a tertiary butyl group as a sterically hindering group. The phenol group may be further substituted with a hydrocarbyl group and/or a bridging group linking to a second aromatic group. Examples of suitable hindered phenol antioxidants include 2,6-di-tert-butylphenol, 4-methyl-2,6-di-tert-butylphenol, 4-ethyl-2,6-di-tert-butylphenol, 4-propyl-2,6-di-tert-butylphenol or 4-butyl-2,6-di-tert-butylphenol, or 4-dodecyl-2,6-di-tert-butylphenol. In one embodiment the hindered phenol antioxidant may be an ester and may include, e.g., Irganox<sup>TM</sup> L-135 available from BASF or an addition product derived from 2,6-di-tert-butylphenol and an alkyl acrylate, wherein the alkyl group may contain about 1 to about 18, or about 2 to about 12, or about 2 to about 8, or about 2 to about 6, or about 4 carbon

atoms. Another commercially available hindered phenol antioxidant may be an ester and may include Ethanol-XM 4716 available from Albemarle Corporation.

Useful antioxidants may include diarylamines and high molecular weight phenols. In an embodiment, the lubricating oil composition may contain a mixture of a diarylamine and a high molecular weight phenol, such that each antioxidant may be present in an amount sufficient to provide up to about 5%, by weight, based upon the final weight of the lubricating oil composition. In an embodiment, the antioxidant may be a mixture of about 0.3 to about 1.5% diarylamine and about 0.4 to about 2.5% high molecular weight phenol, by weight, based upon the final weight of the lubricating oil composition.

Examples of suitable olefins that may be sulfurized to form a sulfurized olefin include propylene, butylene, isobutylene, polyisobutylene, pentene, hexene, heptene, octene, nonene, decene, undecene, dodecene, tridecene, tetradecene, pentadecene, hexadecene, heptadecene, octadecene, nonadecene, eicosene or mixtures thereof. In one embodiment, hexadecene, heptadecene, octadecene, nonadecene, eicosene or mixtures thereof and their dimers, trimers and tetramers are especially useful olefins. Alternatively, the olefin may be a Diels-Alder adduct of a diene such as 1,3-butadiene and an unsaturated ester, such as, butylacrylate.

Another class of sulfurized olefin includes sulfurized fatty acids and their esters. The fatty acids are often obtained from vegetable oil or animal oil and typically contain about 4 to about 22 carbon atoms. Examples of suitable fatty acids and their esters include triglycerides, oleic acid, linoleic acid, palmitoleic acid or mixtures thereof. Often, the fatty acids are obtained from lard oil, tall oil, peanut oil, soybean oil, cottonseed oil, sunflower seed oil or mixtures thereof. Fatty acids and/or ester may be mixed with olefins, such as  $\alpha$ -olefins.

In another alternative embodiment the antioxidant composition also contains a molybdenum-containing antioxidant in addition to the phenolic and/or aminic antioxidants discussed above. When a combination of these three antioxidants is used, preferably the ratio of phenolic to aminic to molybdenum-containing component treat rates is (0 to 3):(0 to 3):(0 to 3).

The one or more antioxidant(s) may be present in ranges about 0 wt. % to about 20 wt. %, or about 0.1 wt. % to about 10 wt. %, or about 1 wt. % to about 5 wt. %, of the lubricating oil composition.

**Antiwear Agents:** The lubricating oil compositions herein also may optionally contain one or more antiwear agents. Examples of suitable antiwear agents include, but are not limited to, a metal thiophosphate; a metal dialkyldithiophosphate; a phosphoric acid ester or salt thereof; a phosphate ester(s); a phosphite; a phosphorus-containing carboxylic ester, ether, or amide; a sulfurized olefin; thiocarbamate-containing compounds including, thiocarbamate esters, alkylene-coupled thiocarbamates, and bis(S-alkyldithiocarbamyl)disulfides; and mixtures thereof. A suitable antiwear agent may be a molybdenum dithiocarbamate. The phosphorus containing antiwear agents are more fully described in European Patent 612 839. The metal in the dialkyl dithiophosphate salts may be an alkali metal, alkaline earth metal, aluminum, lead, tin, molybdenum, manganese, nickel, copper, titanium, or zinc. A useful antiwear agent may be zinc dialkyldithiophosphate.

Further examples of suitable antiwear agents include titanium compounds, tartrates, tartrimides, oil soluble amine salts of phosphorus compounds, sulfurized olefins, phosphi-

tes (such as dibutyl phosphite), phosphonates, thiocarbamate-containing compounds, such as thiocarbamate esters, thiocarbamate amides, thiocarbamic ethers, alkylene-coupled thiocarbamates, and bis(S-alkyldithiocarbamyl) disulfides. The tartrate or tartrimate may contain alkyl-ester groups, where the sum of carbon atoms on the alkyl groups may be at least 8. The antiwear agent may in one embodiment include a citrate.

The antiwear agent may be present in ranges including about 0 wt. % to about 15 wt. %, or about 0.01 wt. % to about 10 wt. %, or about 0.05 wt. % to about 5 wt. %, or about 0.1 wt. % to about 3 wt. % of the lubricating oil composition.

**Boron-Containing Compounds:** The lubricating oil compositions herein may optionally contain one or more boron-containing compounds. Examples of boron-containing compounds include borate esters, borated fatty amines, borated epoxides, borated detergents, and borated dispersants, such as borated succinimide dispersants, as disclosed in U.S. Pat. No. 5,883,057. The boron-containing compound, if present, can be used in an amount sufficient to provide up to about 8 wt. %, about 0.01 wt. % to about 7 wt. %, about 0.05 wt. % to about 5 wt. %, or about 0.1 wt. % to about 3 wt. % of the lubricating oil composition.

**Additional Detergents:** The lubricating oil composition may optionally further comprise one or more neutral, low based, or overbased detergents, and mixtures thereof. Suitable detergent substrates include phenates, sulfur containing phenates, sulfonates, calixarates, salixarates, salicylates, carboxylic acids, phosphorus acids, mono- and/or di-thiophosphoric acids, alkyl phenols, sulfur coupled alkyl phenol compounds, or methylene bridged phenols. Suitable detergents and their methods of preparation are described in greater detail in numerous patent publications, including U.S. Pat. No. 7,732,390 and references cited therein.

The detergent substrate may be salted with an alkali or alkaline earth metal such as, but not limited to, calcium, magnesium, potassium, sodium, lithium, barium, or mixtures thereof. In some embodiments, the detergent is free of barium. In some embodiments, a detergent may contain traces of other metals such as magnesium or calcium in amounts such as 50 ppm or less, 40 ppm or less, 30 ppm or less, 20 ppm or less, or 10 ppm or less. A suitable detergent may include alkali or alkaline earth metal salts of petroleum sulfonic acids and long chain mono- or di-alkylarylsulfonic acids with the aryl group being benzyl, tolyl, and xylyl. Examples of suitable detergents include, but are not limited to, calcium phenates, calcium sulfur containing phenates, calcium sulfonates, calcium calixarates, calcium salixarates, calcium salicylates, calcium carboxylic acids, calcium phosphorus acids, calcium mono- and/or di-thiophosphoric acids, calcium alkyl phenols, calcium sulfur coupled alkyl phenol compounds, calcium methylene bridged phenols, magnesium phenates, magnesium sulfur containing phenates, magnesium sulfonates, magnesium calixarates, magnesium salixarates, magnesium salicylates, magnesium carboxylic acids, magnesium phosphorus acids, magnesium mono- and/or di-thiophosphoric acids, magnesium alkyl phenols, magnesium sulfur coupled alkyl phenol compounds, magnesium methylene bridged phenols, sodium phenates, sodium sulfur containing phenates, sodium sulfonates, sodium calixarates, sodium salixarates, sodium salicylates, sodium carboxylic acids, sodium phosphorus acids, sodium mono- and/or di-thiophosphoric acids, sodium alkyl phenols, sodium sulfur coupled alkyl phenol compounds, or sodium methylene bridged phenols.

Overbased detergent additives are well known in the art and may be alkali or alkaline earth metal overbased detergent additives. Such detergent additives may be prepared by reacting a metal oxide or metal hydroxide with a substrate and carbon dioxide gas. The substrate is typically an acid, for example, an acid such as an aliphatic substituted sulfonic acid, an aliphatic substituted carboxylic acid, or an aliphatic substituted phenol.

The terminology "overbased" relates to metal salts, such as metal salts of sulfonates, carboxylates, and phenates, wherein the amount of metal present exceeds the stoichiometric amount. Such salts may have a conversion level in excess of 100% (i.e., they may comprise more than 100% of the theoretical amount of metal needed to convert the acid to its "normal," "neutral" salt). The expression "metal ratio," often abbreviated as MR, is used to designate the ratio of total chemical equivalents of metal in the overbased salt to chemical equivalents of the metal in a neutral salt according to known chemical reactivity and stoichiometry. In a normal or neutral salt, the metal ratio is one and in an overbased salt, MR, is greater than one. They are commonly referred to as overbased, hyperbased, or superbased salts and may be salts of organic sulfur acids, carboxylic acids, or phenols.

An overbased detergent of the lubricating oil composition may have a total base number (TBN) of about 200 mg KOH/g or greater, or as further examples, about 250 mg KOH/g or greater, or about 350 mg KOH/g or greater, or about 375 mg KOH/g or greater, or about 400 mg KOH/g or greater. The TBN being measured by the method of ASTM D2896.

Examples of suitable overbased detergents include, but are not limited to, overbased calcium phenates, overbased calcium sulfur containing phenates, overbased calcium sulfonates, overbased calcium calixarates, overbased calcium salixarates, overbased calcium salicylates, overbased calcium carboxylic acids, overbased calcium phosphorus acids, overbased calcium mono- and/or di-thiophosphoric acids, overbased calcium alkyl phenols, overbased calcium sulfur coupled alkyl phenol compounds, overbased calcium methylene bridged phenols, overbased magnesium phenates, overbased magnesium sulfur containing phenates, overbased magnesium sulfonates, overbased magnesium calixarates, overbased magnesium salixarates, overbased magnesium salicylates, overbased magnesium carboxylic acids, overbased magnesium phosphorus acids, overbased magnesium mono- and/or di-thiophosphoric acids, overbased magnesium alkyl phenols, overbased magnesium sulfur coupled alkyl phenol compounds, or overbased magnesium methylene bridged phenols.

The overbased calcium phenate detergents have a total base number of at least about 150 mg KOH/g, at least about 225 mg KOH/g, at least about 225 mg KOH/g to about 400 mg KOH/g, at least about 225 mg KOH/g to about 350 mg KOH/g or about 230 mg KOH/g to about 350 mg KOH/g, all as measured by the method of ASTM D2896. When such detergent compositions are formed in an inert diluent, e.g. a process oil, usually a mineral oil, the total base number reflects the basicity of the overall composition including diluent, and any other materials (e.g., promoter, etc.) that may be contained in the detergent composition.

The overbased detergent may have a metal to substrate ratio of from 1.1:1, or from 2:1, or from 4:1, or from 5:1, or from 7:1, or from 10:1. In some embodiments, a detergent is effective at reducing or preventing rust in an engine or other automotive part such as a transmission or gear. The detergent may be present in a lubricating composition at about 0 wt.

% to about 10 wt. %, or about 0.1 wt. % to about 8 wt. %, or about 1 wt. % to about 4 wt. %, or greater than about 4 wt. % to about 8 wt. %.

**Extreme Pressure Agents:** The lubricating oil compositions herein also may optionally contain one or more extreme pressure agents. Extreme Pressure (EP) agents that are soluble in the oil include sulfur- and chlorosulfur-containing EP agents, chlorinated hydrocarbon EP agents and phosphorus EP agents. Examples of such EP agents include chlorinated wax; organic sulfides and polysulfides such as dibenzyl disulfide, bis(chlorobenzyl) disulfide, dibutyl tetrasulfide, sulfurized methyl ester of oleic acid, sulfurized alkyl phenol, sulfurized dipentene, sulfurized terpene, and sulfurized Diels-Alder adducts; phosphosulfurized hydrocarbons such as the reaction product of phosphorus sulfide with turpentine or methyl oleate; phosphorus esters such as the dihydrocarbyl and trihydrocarbyl phosphites, e.g., dibutyl phosphite, diheptyl phosphite, dicyclohexyl phosphite, pentylphenyl phosphite; dipentylphenyl phosphite, tridecyl phosphite, distearyl phosphite and polypropylene substituted phenyl phosphite; metal thiocarbamates such as zinc dioctyldithiocarbamate and barium heptylphenol diacid; amine salts of alkyl and dialkylphosphoric acids, including, for example, the amine salt of the reaction product of a dialkylthiophosphoric acid with propylene oxide; and mixtures thereof.

**Friction Modifiers:** The lubricating oil compositions herein also may optionally contain one or more friction modifiers. Suitable friction modifiers may comprise metal containing and metal-free friction modifiers and may include, but are not limited to, imidazolines, amides, amines, succinimides, alkoxylated amines, alkoxylated ether amines, amine oxides, amidoamines, nitriles, betaines, quaternary amines, imines, amine salts, amino guanadine, alkanol-amides, phosphonates, metal-containing compounds, glycerol esters, sulfurized fatty compounds and olefins, sunflower oil other naturally occurring plant or animal oils, dicarboxylic acid esters, esters or partial esters of a polyol and one or more aliphatic or aromatic carboxylic acids, and the like.

Suitable friction modifiers may contain hydrocarbyl groups that are selected from straight chain, branched chain, or aromatic hydrocarbyl groups or mixtures thereof, and may be saturated or unsaturated. The hydrocarbyl groups may be composed of carbon and hydrogen or hetero atoms such as sulfur or oxygen. The hydrocarbyl groups may range from about 12 to about 25 carbon atoms. In some embodiments the friction modifier may be a long chain fatty acid ester. In another embodiment the long chain fatty acid ester may be a mono-ester, or a di-ester, or a (tri)glyceride. The friction modifier may be a long chain fatty amide, a long chain fatty ester, a long chain fatty epoxide derivatives, or a long chain imidazoline.

Other suitable friction modifiers may include organic, ashless (metal-free), nitrogen-free organic friction modifiers. Such friction modifiers may include esters formed by reacting carboxylic acids and anhydrides with alkanols and generally include a polar terminal group (e.g. carboxyl or hydroxyl) covalently bonded to an oleophilic hydrocarbon chain. An example of an organic ashless nitrogen-free friction modifier is known generally as glycerol monooleate (GMO) which may contain mono-, di-, and tri-esters of oleic acid. Other suitable friction modifiers are described in U.S. Pat. No. 6,723,685, herein incorporated by reference in its entirety.

Aminic friction modifiers may include amines or polyamines. Such compounds can have hydrocarbyl groups

that are linear, either saturated or unsaturated, or a mixture thereof and may contain from about 12 to about 25 carbon atoms. Further examples of suitable friction modifiers include alkoxylated amines and alkoxylated ether amines.

Such compounds may have hydrocarbyl groups that are linear, either saturated, unsaturated, or a mixture thereof. They may contain from about 12 to about 25 carbon atoms. Examples include ethoxylated amines and ethoxylated ether amines.

10 The amines and amides may be used as such or in the form of an adduct or reaction product with a boron compound such as a boric oxide, boron halide, metaborate, boric acid or a mono-, di- or tri-alkyl borate. Other suitable friction modifiers are described in U.S. Pat. No. 6,300,291, herein incorporated by reference in its entirety.

A friction modifier may optionally be present in ranges such as about 0 wt. % to about 10 wt. %, or about 0.01 wt. % to about 8 wt. %, or about 0.1 wt. % to about 4 wt. %.

**Molybdenum-containing component:** The lubricating oil compositions herein also may optionally contain one or more molybdenum-containing compounds. An oil-soluble molybdenum compound may have the functional performance of an antiwear agent, an antioxidant, a friction modifier, or mixtures thereof. An oil-soluble molybdenum compound may include molybdenum dithiocarbamates, molybdenum dialkylthiophosphates, molybdenum dithiophosphinates, amine salts of molybdenum compounds, molybdenum xanthates, molybdenum thioxanthates, molybdenum sulfides, molybdenum carboxylates, molybdenum alkoxides, a trinuclear organo-molybdenum compound, and/or mixtures thereof. The molybdenum sulfides include molybdenum disulfide. The molybdenum disulfide may be in the form of a stable dispersion. In one embodiment the oil-soluble molybdenum compound may be selected from the group consisting of molybdenum dithiocarbamates, molybdenum dialkylthiophosphates, amine salts of molybdenum compounds, and mixtures thereof. In one embodiment the oil-soluble molybdenum compound may be a molybdenum dithiocarbamate.

40 Suitable examples of molybdenum compounds which may be used include commercial materials sold under the trade names such as Molyvan® 822, Molyvan® A, Molyvan® 2000 and Molyvan® 855 from R. T. Vanderbilt Co., Ltd., and Adeka Sakura-Lube® S-165, S-200, S-300, S-310G, S-525, S-600, S-700, and S-710 available from Adeka Corporation, and mixtures thereof. Suitable molybdenum components are described in U.S. Pat. No. 5,650,381; US RE 37,363 E1; US RE 38,929 E1; and US RE 40,595 E1, incorporated herein by reference in their entireties.

55 Additionally, the molybdenum compound may be an acidic molybdenum compound. Included are molybdic acid, ammonium molybdate, sodium molybdate, potassium molybdate, and other alkaline metal molybdates and other molybdenum salts, e.g., hydrogen sodium molybdate,  $\text{MoOCl}_4$ ,  $\text{MoO}_2\text{Br}_2$ ,  $\text{Mo}_2\text{O}_3\text{Cl}_6$ , molybdenum trioxide or similar acidic molybdenum compounds. Alternatively, the compositions can be provided with molybdenum by molybdenum/sulfur complexes of basic nitrogen compounds as described, for example, in U.S. Pat. Nos. 4,263,152; 4,285,822; 4,283,295; 4,272,387; 4,265,773; 4,261,843; 4,259,195 and 4,259,194; and WO 94/06897, incorporated herein by reference in their entireties.

60 Another class of suitable organo-molybdenum compounds are trinuclear molybdenum compounds, such as those of the formula  $\text{Mo}_3\text{S}_k\text{L}_n\text{Q}_x$  and mixtures thereof, wherein S represents sulfur, L represents independently

selected ligands having organo groups with a sufficient number of carbon atoms to render the compound soluble or dispersible in the oil, n is from 1 to 4, k varies from 4 through 7, Q is selected from the group of neutral electron donating compounds such as water, amines, alcohols, phosphines, and ethers, and z ranges from 0 to 5 and includes non-stoichiometric values. At least 21 total carbon atoms may be present among all the ligands' organo groups, such as at least 25, at least 30, or at least 35 carbon atoms. Additional suitable molybdenum compounds are described in U.S. Pat. No. 6,723,685, herein incorporated by reference in its entirety.

The oil-soluble molybdenum compound may be present in an amount sufficient to provide about 0.5 ppm to about 2000 ppm, about 1 ppm to about 700 ppm, about 1 ppm to about 550 ppm, about 5 ppm to about 300 ppm, or about 20 ppm to about 250 ppm of molybdenum.

Transition Metal-containing compounds: In another embodiment, the oil-soluble compound may be a transition metal containing compound or a metalloid. The transition metals may include, but are not limited to, titanium, vanadium, copper, zinc, zirconium, molybdenum, tantalum, tungsten, and the like. Suitable metalloids include, but are not limited to, boron, silicon, antimony, tellurium, and the like.

In an embodiment, an oil-soluble transition metal-containing compound may function as antiwear agents, friction modifiers, antioxidants, deposit control additives, or more than one of these functions. In an embodiment the oil-soluble transition metal-containing compound may be an oil-soluble titanium compound, such as a titanium (IV) alkoxide. Among the titanium containing compounds that may be used in, or which may be used for preparation of the oil-soluble materials of, the disclosed technology are various Ti (IV) compounds such as titanium (IV) oxide; titanium (IV) sulfide; titanium (IV) nitrate; titanium (IV) alkoxides such as titanium methoxide, titanium ethoxide, titanium propoxide, titanium isopropoxide, titanium butoxide, titanium 2-ethylhexoxide; and other titanium compounds or complexes including but not limited to titanium phenates; titanium carboxylates such as titanium (IV) 2-ethyl-1-3-hexanedioate or titanium citrate or titanium oleate; and titanium (IV) (triethanolaminato)isopropoxide. Other forms of titanium encompassed within the disclosed technology include titanium phosphates such as titanium dithiophosphates (e.g., dialkyldithiophosphates) and titanium sulfonates (e.g., alkylbenzenesulfonates), or, generally, the reaction product of titanium compounds with various acid materials to form salts, such as oil-soluble salts. Titanium compounds can thus be derived from, among others, organic acids, alcohols, and glycols. Ti compounds may also exist in dimeric or oligomeric form, containing Ti—O—Ti structures. Such titanium materials are commercially available or can be readily prepared by appropriate synthesis techniques which will be apparent to the person skilled in the art. They may exist at room temperature as a solid or a liquid, depending on the particular compound. They may also be provided in a solution form in an appropriate inert solvent.

In one embodiment, the titanium can be supplied as a Ti-modified dispersant, such as a succinimide dispersant. Such materials may be prepared by forming a titanium mixed anhydride between a titanium alkoxide and a hydrocarbyl-substituted succinic anhydride, such as an alkenyl- (or alkyl) succinic anhydride. The resulting titanate-succinate intermediate may be used directly or it may be reacted with any of a number of materials, such as (a) a polyamine-based succinimide/amide dispersant having free, condens-

able —NH functionality; (b) the components of a polyamine-based succinimide/amide dispersant, i.e., an alkenyl- (or alkyl-) succinic anhydride and a polyamine, (c) a hydroxy-containing polyester dispersant prepared by the reaction of a substituted succinic anhydride with a polyol, aminoalcohol, polyamine, or mixtures thereof. Alternatively, the titanate-succinate intermediate may be reacted with other agents such as alcohols, aminoalcohols, ether alcohols, polyether alcohols or polyols, or fatty acids, and the product thereof either used directly to impart Ti to a lubricant, or else further reacted with the succinic dispersants as described above. As an example, 1 part (by mole) of tetraisopropyl titanate may be reacted with about 2 parts (by mole) of a polyisobutene-substituted succinic anhydride at 140-150° C. for 5 to 6 hours to provide a titanium modified dispersant or intermediate. The resulting material (30 g) may be further reacted with a succinimide dispersant from polyisobutene-substituted succinic anhydride and a polyethylenepolyamine mixture (127 grams+diluent oil) at 150° C. for 1.5 hours, to produce a titanium-modified succinimide dispersant.

Another titanium containing compound may be a reaction product of titanium alkoxide and C<sub>6</sub> to C<sub>25</sub> carboxylic acid. The reaction product may be represented by the following formula:



wherein n is an integer selected from 2, 3 and 4, and R is a hydrocarbyl group containing from about 5 to about 24 carbon atoms, or by the formula:



wherein m+n=4 and n ranges from 1 to 3, R<sub>4</sub> is an alkyl moiety with carbon atoms ranging from 1-8, R<sub>1</sub> is selected from a hydrocarbyl group containing from about 6 to 25 carbon atoms, and R<sub>2</sub> and R<sub>3</sub> are the same or different and are selected from a hydrocarbyl group containing from about 1 to 6 carbon atoms, or the titanium compound may be represented by the formula:



wherein x ranges from 0 to 3, R<sub>1</sub> is selected from a hydrocarbyl group containing from about 6 to 25

carbon atoms, R<sub>2</sub>, and R<sub>3</sub> are the same or different and are selected from a hydrocarbyl group containing from about 1 to 6 carbon atoms, and R<sub>4</sub> is selected from a group consisting of either H, or C6 to C25 carboxylic acid moiety.

Suitable carboxylic acids may include, but are not limited to caproic acid, caprylic acid, lauric acid, myristic acid, palmitic acid, stearic acid, arachidic acid, oleic acid, erucic acid, linoleic acid, linolenic acid, cyclohexanecarboxylic acid, phenylacetic acid, benzoic acid, neodecanoic acid, and the like.

In an embodiment the oil soluble titanium compound may be present in the lubricating oil composition in an amount to provide from 0 to 3000 ppm titanium by weight or 25 to about 1500 ppm titanium by weight or about 35 ppm to 500 ppm titanium by weight or about 50 ppm to about 300 ppm.

Viscosity Index Improvers: The lubricating oil compositions herein also may optionally contain one or more viscosity index improvers. Suitable viscosity index improvers may include polyolefins, olefin copolymers, ethylene/propylene copolymers, polyisobutenes, hydrogenated styrene-isoprene polymers, styrene/maleic ester copolymers, hydrogenated styrene/butadiene copolymers, hydrogenated isoprene polymers, alpha-olefin maleic anhydride copolymers, polymethacrylates, polyacrylates, polyalkyl styrenes, hydrogenated alkenyl aryl conjugated diene copolymers, or mixtures thereof. Viscosity index improvers may include star polymers and suitable examples are described in US Publication No. 20120101017A1.

The lubricating oil compositions herein also may optionally contain one or more dispersant viscosity index improvers in addition to a viscosity index improver or in lieu of a viscosity index improver. Suitable viscosity index improvers may include functionalized polyolefins, for example, ethylene-propylene copolymers that have been functionalized with the reaction product of an acylating agent (such as maleic anhydride) and an amine; polymethacrylates functionalized with an amine, or esterified maleic anhydride-styrene copolymers reacted with an amine.

The total amount of viscosity index improver and/or dispersant viscosity index improver may be about 0 wt. % to about 20 wt. %, about 0.1 wt. % to about 15 wt. %, about 0.1 wt. % to about 12 wt. %, or about 0.5 wt. % to about 10 wt. %, of the lubricating oil composition.

Other Optional Additives: Other additives may be selected to perform one or more functions required of a lubricating fluid. Further, one or more of the mentioned additives may be multi-functional and provide functions in addition to or other than the function prescribed herein.

A lubricating oil composition according to the present disclosure may optionally comprise other performance additives. The other performance additives may be in addition to specified additives of the present disclosure and/or may comprise one or more of metal deactivators, viscosity index improvers, detergents, ashless TBN boosters, friction modifiers, antiwear agents, corrosion inhibitors, rust inhibitors, dispersants, dispersant viscosity index improvers, extreme pressure agents, antioxidants, foam inhibitors, demulsifiers, emulsifiers, pour point depressants, seal swelling agents and mixtures thereof. Typically, fully-formulated lubricating oil will contain one or more of these performance additives.

Suitable metal deactivators may include derivatives of benzotriazoles (typically tolyltriazole), dimercaptotriadiazole derivatives, 1,2,4-triazoles, benzimidazoles, 2-alkyldithiobenzimidazoles, or 2-alkyldithiobenzothiazoles; foam inhibitors including copolymers of ethyl acrylate and 2-ethylhexylacrylate and optionally vinyl acetate; demulsifiers

including trialkyl phosphates, polyethylene glycols, polyethylene oxides, polypropylene oxides and (ethylene oxide-propylene oxide) polymers; pour point depressants including esters of maleic anhydride-styrene, polymethacrylates, polyacrylates or polyacrylamides.

Suitable foam inhibitors include silicon-based compounds, such as siloxane.

Suitable pour point depressants may include polymethylmethacrylates or mixtures thereof. Pour point depressants may be present in an amount sufficient to provide from about 0 wt. % to about 1 wt. %, about 0.01 wt. % to about 0.5 wt. %, or about 0.02 wt. % to about 0.04 wt. % based upon the final weight of the lubricating oil composition.

Suitable rust inhibitors may be a single compound or a mixture of compounds having the property of inhibiting corrosion of ferrous metal surfaces. Non-limiting examples of rust inhibitors useful herein include oil-soluble high molecular weight organic acids, such as 2-ethylhexanoic acid, lauric acid, myristic acid, palmitic acid, oleic acid, linoleic acid, linolenic acid, behenic acid, and cerotic acid, as well as oil-soluble polycarboxylic acids including dimer and trimer acids, such as those produced from tall oil fatty acids, oleic acid, and linoleic acid. Other suitable corrosion inhibitors include long-chain alpha, omega-dicarboxylic acids in the molecular weight range of about 600 to about 3000 and alkenylsuccinic acids in which the alkenyl group contains about 10 or more carbon atoms such as, tetrapropenylsuccinic acid, tetradecenylsuccinic acid, and hexadecenylsuccinic acid. Another useful type of acidic corrosion inhibitors are the half esters of alkenyl succinic acids having about 8 to about 24 carbon atoms in the alkenyl group with alcohols such as the polyglycols. The corresponding half amides of such alkenyl succinic acids are also useful. A useful rust inhibitor is a high molecular weight organic acid.

The rust inhibitor, if present, can be used in an amount sufficient to provide about 0 wt. % to about 5 wt. %, about 0.01 wt. % to about 3 wt. %, about 0.1 wt. % to about 2 wt. %, based upon the final weight of the lubricating oil composition.

In general terms, a suitable lubricant including the detergent metals herein may include additive components in the ranges listed in the following table.

TABLE 2

| Suitable Lubricating Compositions      |                                 |                                 |
|----------------------------------------|---------------------------------|---------------------------------|
| Component                              | Wt. %<br>(Suitable Embodiments) | Wt. %<br>(Suitable Embodiments) |
| Detergent Systems                      | 0.02-5.0                        | 0.2-2.0                         |
| Dispersant(s)                          | 0-8.0                           | 1-6.0                           |
| Antioxidant(s)                         | 0.1-5.0                         | 0.01-3.0                        |
| Other Detergent(s)                     | 0.0-15.0                        | 0.2-8.0                         |
| Ashless TBN booster(s)                 | 0.0-1.0                         | 0.01-0.5                        |
| Corrosion inhibitor(s)                 | 0.0-5.0                         | 0.0-2.0                         |
| Metal dihydrocarbyldithiophosphate(s)  | 0.0-6.0                         | 0.1-4.0                         |
| Ash-free phosphorus compound(s)        | 0.0-6.0                         | 0.0-4.0                         |
| Antifoaming agent(s)                   | 0.0-5.0                         | 0.001-0.15                      |
| Antiwear agent(s)                      | 0.0-1.0                         | 0.0-0.8                         |
| Pour point depressant(s)               | 0.0-5.0                         | 0.01-1.5                        |
| Viscosity index improver(s)            | 0.0-25.0                        | 0.1-15.0                        |
| Dispersant viscosity index improver(s) | 0.0-10.0                        | 0.0-5.0                         |
| Friction modifier(s)                   | 0.00-5.0                        | 0.01-2.0                        |
| Base oil                               | Balance                         | Balance                         |
| Total                                  | 100                             | 100                             |

The percentages of each component above represent the weight percent of each component, based upon the weight of

the final lubricating oil composition. The remainder of the lubricating oil composition consists of one or more base oils. Additives used in formulating the compositions described herein may be blended into the base oil individually or in various sub-combinations. However, it may be suitable to blend all of the components concurrently using an additive concentrate (i.e., additives plus a diluent, such as a hydrocarbon solvent). Fully formulated lubricants conventionally contain an additive package, referred to herein as a dispersant/inhibitor package or DI package, that will supply the characteristics that are required in the formulation.

#### Definitions

For purposes of this disclosure, the chemical elements are identified in accordance with the Periodic Table of the Elements, CAS version, Handbook of Chemistry and Physics, 75th Ed. Additionally, general principles of organic chemistry are described in "Organic Chemistry", Thomas Sorrell, University Science Books, Sausalito: 1999, and "March's Advanced Organic Chemistry", 5th Ed., Ed.: Smith, M. B. and March, J., John Wiley & Sons, New York: 2001, the entire contents of which are hereby incorporated by reference.

As described herein, compounds may optionally be substituted with one or more substituents, such as illustrated generally above, or as exemplified by particular classes, subclasses, and species of the disclosure.

Unless otherwise apparent from the context, the term "major amount" is understood to mean an amount greater than or equal to 50 weight percent, for example, from about 80 to about 98 weight percent relative to the total weight of the composition. Moreover, as used herein, the term "minor amount" is understood to mean an amount less than 50 weight percent relative to the total weight of the composition.

As used herein, the term "hydrocarbyl group" or "hydrocarbyl" is used in its ordinary sense, which is well-known to those skilled in the art. Specifically, it refers to a group having a carbon atom directly attached to the remainder of a molecule and having a predominantly hydrocarbon character. Examples of hydrocarbyl groups include: (1) hydrocarbon substituents, that is, aliphatic (e.g., alkyl or alkenyl), alicyclic (e.g., cycloalkyl, cycloalkenyl) substituents, and aromatic-, aliphatic-, and alicyclic-substituted aromatic substituents, as well as cyclic substituents wherein the ring is completed through another portion of the molecule (e.g., two substituents together form an alicyclic radical); (2) substituted hydrocarbon substituents, that is, substituents containing non-hydrocarbon groups which, in the context of the description herein, do not alter the predominantly hydrocarbon substituent (e.g., halo (especially chloro and fluoro), hydroxy, alkoxy, mercapto, alkylmercapto, nitro, nitroso, amino, alkylamino, and sulfoxyl); (3) hetero-substituents, that is, substituents which, while having a predominantly hydrocarbon character, in the context of this description, contain other than carbon in a ring or chain otherwise composed of carbon atoms. Hetero-atoms include sulfur, oxygen, nitrogen, and encompass substituents such as pyridyl, furyl, thienyl, and imidazolyl. In general, no more than two, or as a further example, no more than one, non-hydrocarbon substituent will be present for every ten carbon atoms in the hydrocarbyl group; in some embodiments, there will be no non-hydrocarbon substituent in the hydrocarbyl group.

As used herein the term "aliphatic" encompasses the terms alkyl, alkenyl, alkynyl, each of which being optionally substituted as set forth below.

As used herein, an "alkyl" group refers to a saturated 5 aliphatic hydrocarbon group containing 1-12 (e.g., 1-8, 1-6, or 1-4) carbon atoms. An alkyl group can be straight or branched. Examples of alkyl groups include, but are not limited to, methyl, ethyl, propyl, isopropyl, butyl, isobutyl, sec-butyl, tert-butyl, n-pentyl, n-heptyl, or 2-ethylhexyl. An 10 alkyl group can be substituted (i.e., optionally substituted) with one or more substituents such as halo, phospho, cycloaliphatic [e.g., cycloalkyl or cycloalkenyl], heterocycloaliphatic [e.g., heterocycloalkyl or heterocycloalkenyl], aryl, heteroaryl, alkoxy, aroyl, heteroaroyl, acyl [e.g., (aliphatic) 15 carbonyl, (cycloaliphatic)carbonyl, or (heterocycloaliphatic) carbonyl], nitro, cyano, amido [e.g., (cycloalkylalkyl)carbonylamino, arylcarbonylamino, aralkylcarbonylamino, (heterocycloalkyl) carbonylamino, heteroarylcarbonylamino, heteroaralkyl carbonylamino alkylaminocarbonyl, cycloalkylaminocarbonyl, 20 heterocycloalkylaminocarbonyl, arylaminocarbonyl, or heteroarylamino carbonyl], amino [e.g., aliphaticamino, cycloaliphatic amino, or heterocycloaliphaticamino], sulfonyl [e.g., aliphatic-SO<sub>2</sub>—], sulfinyl, sulfanyl, sulfoxyl, urea, 25 thiourea, sulfamoyl, sulfamide, oxo, carboxy, carbamoyl, cycloaliphaticoxy, heterocyclo aliphaticoxy, aryloxy, heteroaryloxy, aralkyloxy, heteroarylalkoxy, alkoxy carbonyl, alkyl carbonyloxy, or hydroxy. Without limitation, some examples of substituted alkyls include carboxyalkyl (such as 30 HOOC-alkyl, alkoxy carbonylalkyl, and alkylcarbonyloxy-alkyl), cyanoalkyl, hydroxyalkyl, alkoxyalkyl, acylalkyl, aralkyl, (alkoxyaryl)alkyl, (sulfonylamino) alkyl (such as (alkyl-SO<sub>2</sub>-amino)alkyl), aminoalkyl, amidoalkyl, (cycloaliphatic)alkyl, or haloalkyl.

As used herein, an "alkenyl" group refers to an aliphatic 35 carbon group that contains 2-8 (e.g., 2-12, 2-6, or 2-4) carbon atoms and at least one double bond. Like an alkyl group, an alkenyl group can be straight or branched. Examples of an alkenyl group include, but are not limited to 40 allyl, isoprenyl, 2-butenyl, and 2-hexenyl. An alkenyl group can be optionally substituted with one or more substituents such as halo, phospho, cycloaliphatic [e.g., cycloalkyl or cycloalkenyl], heterocycloaliphatic [e.g., heterocycloalkyl or hetero cycloalkenyl], aryl, heteroaryl, alkoxy, aroyl, heteroaroyl, acyl [e.g., (aliphatic) carbonyl, (cycloaliphatic) carbonyl, or (heterocycloaliphatic)carbonyl], nitro, cyano, 45 amido [e.g., (cycloalkylalkyl)carbonylamino, arylcarbonylamino, aralkylcarbonylamino, (hetero cycloalkyl) carbonylamino, (heterocyclo alkylalkyl) carbonylamino, heteroarylcarbonylamino, heteroaralkylcarbonylamino 50 alkylamino carbonyl, cycloalkylaminocarbonyl, hetero cyclo alkylaminocarbonyl, arylaminocarbonyl, or heteroarylamino carbonyl], amino [e.g., aliphaticamino, cycloaliphaticamino, heterocyclo aliphaticamino, or aliphatic sulfonylamino], sulfonyl [e.g., alkyl-SO<sub>2</sub>—, cycloaliphatic-SO<sub>2</sub>—, or aryl-SO<sub>2</sub>—], sulfinyl, sulfanyl, sulfoxyl, urea, thiourea, sulfamoyl, sulfamide, oxo, carboxy, carbamoyl, cycloaliphaticoxy, heterocycloaliphaticoxy, aryloxy, heteroaryloxy, aralkyloxy, heteroaralkoxy, alkoxy carbonyl, 55 alkylcarbonyloxy, or hydroxy. Without limitation, some examples of substituted alkenyls include cyanoalkenyl, alkoxyalkenyl, acylalkenyl, hydroxyl alkenyl, aralkenyl, (alkoxyaryl) alkenyl, (sulfonylamino)alkenyl (such as (alkyl-SO<sub>2</sub>-amino) alkenyl), aminoalkenyl, amidoalkenyl, (cycloaliphatic)alkenyl, or haloalkenyl.

As used herein, an "alkynyl" group refers to an aliphatic 60 carbon group that contains 2-8 (e.g., 2-12, 2-6, or 2-4)

carbon atoms and has at least one triple bond. An alkynyl group can be straight or branched. Examples of an alkynyl group include, but are not limited to, propargyl and butynyl. An alkynyl group can be optionally substituted with one or more substituents such as aroyl, heteroaroyl, alkoxy, cycloalkyloxy, heterocycloalkyloxy, aryloxy, heteroaryloxy, aralkyl oxy, nitro, carboxy, cyano, halo, hydroxy, sulfo, mercapto, sulfanyl [e.g., aliphatic sulfanyl or cycloaliphatic sulfanyl], sulfinyl [e.g., aliphatic sulfinyl or cycloaliphatic sulfinyl], sulfonyl [e.g., aliphatic  $\text{SO}_2-$  or cycloaliphatic  $\text{SO}_2-$ ], amido [e.g., aminocarbonyl, alkylaminocarbonyl, alkylcarbonylamino, cyclo alkylaminocarbonyl, heterocycloalkylaminocarbonyl, cycloalkylcarbonylamino, arylamino carbonyl, arylcarbonylamino, aralkylcarbonylamino, (heterocycloalkyl) carbonylamino, (cycloalkylalkyl) carbonylamino, heteroaralkylcarbonylamino, heteroaryl carbonylamino or heteroaryl amino carbonyl], urea, thiourea, sulfamoyl, sulfamide, alkoxy carbonyl, alkyl carbonyloxy, cyclo aliphatic, heterocycloaliphatic, aryl, heteroaryl, acyl [e.g., (cycloaliphatic) carbonyl or (hetero cyclo aliphatic) carbonyl], amino [e.g., aliphatic amino], sulfoxyl, oxo, carboxyl, carbamoyl, (cycloaliphatic) oxy, (heterocyclo aliphatic) oxy, or (heteroaryl) alkoxy.

As used herein, an "amino" group refers to  $-\text{NR}^X\text{R}^Y$  wherein each of  $\text{R}^X$  and  $\text{R}^Y$  is independently hydrogen, alkyl, cycloalkyl, (cycloalkyl)alkyl, aryl, aralkyl, heterocycloalkyl, (heterocycloalkyl)alkyl, heteroaryl, carboxyl, sulfanyl, sulfinyl, sulfonyl, (alkyl)carbonyl, (cycloalkyl)carbonyl, ((cycloalkyl)alkyl)carbonyl, arylcarbonyl, (aralkyl)carbonyl, (heterocyclo alkyl) carbonyl, ((heterocycloalkyl)alkyl)carbonyl, (heteroaryl)carbonyl, or (heteroaralkyl) carbonyl, each of which being defined herein and being optionally substituted. Examples of amino groups include alkylamino, dialkylamino, or arylamino. When the term "amino" is not the terminal group (e.g., alkylcarbonylamino), it is represented by  $-\text{NR}^X-$ .  $\text{R}^X$  has the same meaning as defined above.

As used herein, a "cycloalkyl" group refers to a saturated carbocyclic mono- or bicyclic (fused or bridged) ring of 3-10 (e.g., 5-10) carbon atoms. Examples of cycloalkyl groups include cyclopropyl, cyclobutyl, cyclopentyl, cyclohexyl, cycloheptyl, adamantyl, norbornyl, cubyl, octahydroindenyl, decahydro-naphthyl, bicyclo[3.2.1]octyl, bicyclo[2.2.2]octyl, bicyclo[3.3.1]nonyl, bicyclo[3.3.2.]decyl, bicyclo[2.2.2]octyl, adamantyl, or ((aminocarbonyl)cycloalkyl)cycloalkyl.

As used herein, a "heterocycloalkyl" group refers to a 3-10 membered mono- or bicyclic (fused or bridged) (e.g., 5- to 10-membered mono- or bicyclic) saturated ring structure, in which one or more of the ring atoms is a heteroatom (e.g., N, O, S, or combinations thereof). Examples of a heterocycloalkyl group include piperidyl, piperazyl, tetrahydropyranyl, tetrahydrofuryl, 1,4-dioxolanyl, 1,4-dithianyl, 1,3-dioxolanyl, oxazolidyl, isoxazolidyl, morpholinyl, thiomorpholyl, octahydrobenzfuryl, octahydrochromenyl, octahydrothio chromenyl, octahydroindolyl, octahydronaphthyl, decahydroquinolinyl, octahydrobenzo[b]thiophenyl, 2-oxa-bicyclo[2.2.2]octyl, 1-aza-bicyclo[2.2.2]octyl, 3-aza-bicyclo[3.2.1]octyl, and 2,6-dioxa-tricyclo[3.3.1.0]nonyl. A monocyclic heterocycloalkyl group can be fused with a phenyl moiety to form structures, such as tetrahydroisoquinoline, which would be categorized as heteroaryls.

A "heteroaryl" group, as used herein, refers to a monocyclic, bicyclic, or tricyclic ring system having 4 to 15 ring atoms wherein one or more of the ring atoms is a heteroatom

(e.g., N, O, S, or combinations thereof) and in which the monocyclic ring system is aromatic or at least one of the rings in the bicyclic or tricyclic ring systems is aromatic. A heteroaryl group includes a benzofused ring system having 2 to 3 rings. For example, a benzofused group includes benzo fused with one or two 4 to 8 membered heterocycloaliphatic moieties (e.g., indolizyl, indolyl, isoindolyl, 3H-indolyl, indolinyl, benzo[b]furyl, benzo[b]thiophenyl, quinolinyl, or isoquinolinyl). Some examples of heteroaryl are pyridyl, 1H-indazolyl, furyl, pyrrolyl, thienyl, thiazolyl, oxazolyl, imidazolyl, tetrazolyl, benzofuryl, isoquinolinyl, benzthiazolyl, xanthene, thioxanthene, phenothiazine, dihydroindole, benzo[1,3]dioxole, benzo[b]furyl, benzo[b] thiophenyl, indazolyl, benzimidazolyl, benzthiazolyl, puryl, cinnolyl, quinolyl, quinazolyl, cinnolyl, phthalazyl, quinazolyl, quinoxalyl, isoquinolyl, 4H-quinolizyl, benzo-1,2,5-thiadiazolyl, or 1,8-naphthyridyl.

Without limitation, monocyclic heteroaryls include furyl, thiophenyl, 2H-pyrrolyl, pyrrolyl, oxazolyl, thiazolyl, imidazolyl, pyrazolyl, isoxazolyl, isothiazolyl, 1,3,4-thiadiazolyl, 2H-pyranyl, 4H-pranyl, pyridyl, pyridazyl, pyrimidyl, pyrazolyl, pyrazyl, or 1,3,5-triazyl. Monocyclic heteroaryls are numbered according to standard chemical nomenclature.

Without limitation, bicyclic heteroaryls include indolizyl, indolyl, isoindolyl, 3H-indolyl, indolinyl, benzo[b]furyl, benzo[b]thiophenyl, quinolinyl, isoquinolinyl, indolizinyl, isoindolyl, indolyl, benzo[b]furyl, bexo[b]thiophenyl, indazolyl, benzimidazolyl, benzthiazolyl, purinyl, 4H-quinolizyl, quinolyl, isoquinolyl, cinnolyl, phthalazyl, quinazolyl, quinoxalyl, 1,8-naphthyridyl, or pteridyl. Bicyclic heteroaryls are numbered according to standard chemical nomenclature.

As used herein, the term "treat rate" refers to the weight percent of a component in the lubricating and cooling fluids.

The weight average molecular weight ( $M_w$ ) and the number average molecular weight ( $M_n$ ) may be determined with a gel permeation chromatography (GPC) instrument obtained from Waters or the like instrument and the data processed with Waters Empower Software or the like software. The GPC instrument may be equipped with a Waters Separations Module and Waters Refractive Index detector (or the like optional equipment). The GPC operating conditions may include a guard column, 4 Agilent PLgel columns (length of 300 $\times$ 7.5 mm; particle size of 5 $\mu$ , and pore size ranging from 100-10000  $\text{\AA}$ ) with the column temperature at about 40° C. Un-stabilized HPLC grade tetrahydrofuran (THF) may be used as solvent, at a flow rate of 1.0 mL/min. The GPC instrument may be calibrated with commercially available poly(methyl methacrylate) (PMMA) standards having a narrow molecular weight distribution ranging from 960-1,568,000 g/mol. The calibration curve can be extrapolated for samples having a mass less than 500 g/mol. Samples and PMMA standards can be in dissolved in THF and prepared at concentration of 0.1 to 0.5 wt. % and used without filtration. GPC measurements are also described in U.S. Pat. No. 5,266,223, which is incorporated herein by reference. The GPC method additionally provides molecular weight distribution information; see, for example, W. W. Yau, J. J. Kirkland and D. D. Bly, "Modern Size Exclusion Liquid Chromatography", John Wiley and Sons, New York, 1979, also incorporated herein by reference.

### Example

A better understanding of the present disclosure and its many advantages may be clarified with the following example. The following example is illustrative and not limiting thereof in either scope or spirit. Those skilled in the

art will readily understand that variations of the components, methods, steps, and devices described in these examples can be used. Unless noted otherwise or apparent from the context of discussion in the Example below and throughout this disclosure, all percentages, ratios, and parts noted in this disclosure are by weight.

Inventive and Comparative lubricating compositions were subjected to the Sequence IX low-speed pre-ignition (LSPI) test of ASTM D8291-21a. The Inventive and Comparative lubricating compositions included detergent systems, anti-wear systems, and antifoam additives to provide the lubricant elementals as set forth in Table 3 below. Each lubricating composition of this Example included the same amounts of other additives including dispersants, antioxidants, organo-molybdenum additives, ashless antiwear additives, pour point dispersants, and viscosity index modifier. The additives were blended in identical base oils including a blend of API Group II and API Group III base oils. Accordingly, the only material change in each of the lubricants were the additives in the detergent system and the antifoam amounts.

levels of phosphorus shown in Table 3. On the other hand, Inventive lubricants with the lower levels of phosphorus achieved passing Sequence IX LSPI requirements when the noted ratios of phosphorus-to-calcium SASH and/or calcium SASH-to-silicon were maintained.

It is noted that, as used in this specification and the appended claims, the singular forms "a," "an," and "the," include plural referents unless expressly and unequivocally limited to one referent. Thus, for example, reference to "an antioxidant" includes two or more different antioxidants. As used herein, the term "include" and its grammatical variants are intended to be non-limiting, such that recitation of items in a list is not to the exclusion of other like items that can be substituted or added to the listed items

For the purposes of this specification and appended claims, unless otherwise indicated, all numbers expressing quantities, percentages or proportions, and other numerical values used in the specification and claims, are to be understood as being modified in all instances by the term "about." Accordingly, unless indicated to the contrary, the numerical parameters set forth in the following specification

TABLE 3

| Lubricating Composition |                  |                  |                  |                  |                  |
|-------------------------|------------------|------------------|------------------|------------------|------------------|
| Component Base Oil      | C-1 Group II/III | C-2 Group II/III | C-3 Group II/III | I-1 Group II/III | I-2 Group II/III |
| Calcium                 | 780 ppm          | 1190 ppm         | 988 ppm          | 500 ppm          | 500 ppm          |
| Magnesium               | 712 ppm          | 442 ppm          | 573 ppm          | 902 ppm          | 902 ppm          |
| Phosphorus              | 236 ppm          | 234 ppm          | 234 ppm          | 224 ppm          | 230 ppm          |
| Silicon                 | 7 ppm            | 12 ppm           | 12 ppm           | 7 ppm            | 12 ppm           |
| Ca SASH*                | 0.27 wt. %       | 0.40 wt. %       | 0.34 wt. %       | 0.17 wt. %       | 0.17 wt. %       |
| Mg SASH*                | 0.36 wt. %       | 0.22 wt. %       | 0.29 wt. %       | 0.46 wt. %       | 0.46 wt. %       |
| Total Detergent SASH*   | 0.63 wt. %       | 0.63 wt. %       | 0.63 wt. %       | 0.63 wt. %       | 0.63 wt. %       |
| Phosphorus to Ca-SASH** | 0.09             | 0.06             | 0.07             | 0.13             | 0.13             |
| Ca-SASH to silicon      | 385.7            | 333.3            | 283.3            | 242.9            | 141.7            |

\*Calculated as described herein

\*\*wt. % phosphorus/wt. % Ca-SASH (i.e., C1 is (236 ppm/10000)/0.27)

\*\*\*wt. % Ca-SASH/wt. % silicon (i.e., C1 is 0.27/(7 ppm/10000))

In the detergent systems of Table 3, the calcium was provided by a calcium sulfonate detergent with a TBN of about 307 (a neat TBN of 413) and the magnesium was provided by a magnesium sulfonate with a TBN of 400 (a neat TBN of 680). The phosphorus was provided by a zinc dialkyldithiophosphate with alkyl groups provided by a secondary alcohol. The silicon was provided by polydimethylsiloxane antifoam agent.

Each of the Inventive and Comparative lubricating compositions of Table 3 were subjected to the Sequence IX low-speed pre-ignition (LSPI) test of ASTM D8291-21a. Results are provided in Table 4 below.

TABLE 4

| LSPI Events                 | Sequence IX LSPI |       |      |      |      |
|-----------------------------|------------------|-------|------|------|------|
|                             | C-1              | C-2   | C-3  | I-1  | I-2  |
| Average LSPI events (5 max) | 6.78             | 30.52 | 8.28 | 0.53 | 0.07 |
| Maximum LSPI events (8 max) | 8.89             | 30.52 | 8.28 | 1.38 | 0.07 |
| Pass/Fail                   | FAIL             | FAIL  | FAIL | PASS | PASS |

As shown in Table 4 above, none of the comparative fluids was capable of achieving passing Sequence IX LSPI requirements for passenger car motor oils with the lower

and attached claims are approximations that can vary depending upon the desired properties sought to be obtained by the present disclosure. At the very least, and not as an attempt to limit the application of the doctrine of equivalents to the scope of the claims, each numerical parameter should at least be construed in light of the number of reported significant digits and by applying ordinary rounding techniques.

It is to be understood that each component, compound, substituent or parameter disclosed herein is to be interpreted as being disclosed for use alone or in combination with one or more of each and every other component, compound, substituent or parameter disclosed herein.

It is further understood that each range disclosed herein is to be interpreted as a disclosure of each specific value within the disclosed range that has the same number of significant digits. Thus, for example, a range from 1 to 4 is to be interpreted as an express disclosure of the values 1, 2, 3 and 4 as well as any range of such values.

It is further understood that each lower limit of each range disclosed herein is to be interpreted as disclosed in combination with each upper limit of each range and each specific value within each range disclosed herein for the same component, compounds, substituent or parameter. Thus, this disclosure to be interpreted as a disclosure of all ranges derived by combining each lower limit of each range with

each upper limit of each range or with each specific value within each range, or by combining each upper limit of each range with each specific value within each range. That is, it is also further understood that any range between the endpoint values within the broad range is also discussed herein. Thus, a range from 1 to 4 also means a range from 1 to 3, 1 to 2, 2 to 4, 2 to 3, and so forth.

Furthermore, specific amounts/values of a component, compound, substituent or parameter disclosed in the description or an example is to be interpreted as a disclosure of either a lower or an upper limit of a range and thus can be combined with any other lower or upper limit of a range or specific amount/value for the same component, compound, substituent or parameter disclosed elsewhere in the application to form a range for that component, compound, substituent or parameter.

While particular embodiments have been described, alternatives, modifications, variations, improvements, and substantial equivalents that are or can be presently unforeseen can arise to applicants or others skilled in the art. Accordingly, the appended claims as filed and as they can be amended are intended to embrace all such alternatives, modifications variations, improvements, and substantial equivalents.

What is claimed is:

1. A lubricating composition for a spark-ignition engine, the lubricating composition comprising:

one or more base oils of lubricating viscosity;

one or more phosphorus-containing additives providing no more than about 500 ppm of phosphorus to the lubricating composition;

a detergent system providing one or more overbased calcium-containing detergents and optionally one or more magnesium-containing detergents, and wherein the detergent system is substantially free of sodium-containing detergents;

one or more silicon-containing compounds providing about 3 to about 20 ppm silicon to the lubricating composition;

wherein the lubricating composition includes a calcium content providing no more than 0.19 weight percent of calculated calcium sulfated ash content;

a weight ratio of phosphorus content to calcium sulfated ash content of at least about 0.1;

wherein about 30 weight percent or less of total calculated SASH content is provided by the calcium sulfated ash content;

wherein the overbased calcium-containing detergent has a total base number (TBN) of at least about 250 mg KOH/g as determined by ASTM D2896; and wherein a weight ratio of calcium sulfated ash content to silicon content is about 250 or less.

2. The lubricating composition of claim 1, wherein the weight ratio of the phosphorus content to the calcium sulfated ash content is about 0.1 to about 0.3.

3. The lubricating composition of claim 2, wherein the lubricating composition has a total calculated sulfated ash content (SASH) of about 1 weight percent or less.

4. The lubricating composition of claim 1, wherein the lubricating composition has a total calculated sulfated ash content (SASH) of about 0.8 weight percent or less.

5. The lubricating composition of claim 1, wherein the lubricating composition has a total calculated sulfated ash content (SASH) of about 0.7 weight percent or less.

6. The lubricating composition of claim 1, wherein the one or more silicon-containing compounds provide about 5 to about 15 ppm silicon.

7. The lubricating composition of claim 1, wherein the silicon-containing compound is selected from organosilane compounds, fluorosilicone compounds, polydimethylsiloxane compounds, phenyl-methyl polysiloxane compounds, linear siloxane compounds, cyclic siloxane compounds, branched siloxane compounds, silicone polymers and copolymers, organo-silicone copolymers, silicone oil, or combinations thereof.

8. The lubricating composition of claim 1, wherein the detergent system includes the calcium-containing detergent and the magnesium-containing detergent.

9. The lubricating composition of claim 1, wherein the detergent system includes calcium sulfonate and optionally magnesium sulfonate.

10. The lubricating composition of claim 9, wherein the calcium sulfonate and the optional magnesium sulfonate are each overbased and each having a total base number (TBN) of at least about 250 mg KOH/g as determined by ASTM D2896.

11. The lubricating compositions of claim 1, wherein the detergent system is free of phenate-based detergents.

12. The lubricating composition of claim 1, wherein the one or more base oils of lubricating viscosity are selected from API Group I base oils, API Group II base oils, API Group III base oils, or combinations thereof.

13. The lubricating composition of claim 1, wherein the one or more base oils of lubricating viscosity are selected from API Group I base oils, API Group II base oils, or combinations thereof.

14. The lubricating composition of claim 1, wherein the lubricating composition exhibits no more than 5 average events pursuant to a Sequence IX low speed pre-ignition test of ASTM D8291 and/or exhibits no more than 8 maximum events pursuant to the Sequence IX low speed pre-ignition test of ASTM D8291.

15. The lubricating composition of claim 1, wherein the one or more phosphorus-containing additives provide about 200 to about 400 ppm phosphorus.

16. A method of lubricating a spark-ignition engine, the method comprising:

lubricating the crankcase of a spark-ignition engine with a lubricating composition;

wherein the lubricating composition includes (i) one or more base oils of lubricating viscosity; (ii) one or more phosphorus-containing additives providing no more than about 500 ppm of phosphorus to the lubricating composition; (iii) a detergent system providing one or more overbased calcium-containing detergents and optionally one or more magnesium-containing detergents, and wherein the detergent system is substantially free of sodium-containing detergents; (iv) one or more silicon-containing compounds providing about 3 to about 20 ppm silicon to the lubricating composition; (v) wherein the lubricating composition includes a calcium content providing no more than 0.19 weight percent calculated calcium sulfated ash content; (vi) a weight ratio of phosphorus content to calcium sulfated ash content of at least about 0.1; and wherein about 30 weight percent or less of total calculated SASH content is provided by the calcium sulfated ash content;

wherein the overbased calcium-containing detergent has a total base number (TBN) of at least about 250 mg KOH/g as determined by ASTM D2896; and wherein a weight ratio of calcium sulfated ash content to silicon content is about 250 or less; and wherein the lubricating composition exhibits no more than 5 average events pursuant to a Sequence IX low

speed pre-ignition test of ASTM D8291 and/or exhibits no more than 8 maximum events pursuant to the Sequence IX low speed pre-ignition test of ASTM D8291.

**17.** The method of claim 16, wherein the weight ratio of 5 the phosphorus content to the calcium sulfated ash content is about 0.1 to about 0.3.

**18.** The method of claim 16, wherein the lubricating composition further includes one or more silicon-containing compounds providing about 3 to about 20 ppm silicon to the 10 lubricating composition.

\* \* \* \* \*